



US005338648A

**United States Patent** [19]

Kojima et al.

[11] Patent Number: **5,338,648**[45] Date of Patent: **Aug. 16, 1994**[54] **PROCESS OF PROCESSING SILVER HALIDE PHOTOGRAPHIC MATERIAL AND PHOTOGRAPHIC PROCESSING COMPOSITION HAVING A FIXING ABILITY**[75] Inventors: **Tetsuro Kojima; Nobuo Watanabe,** both of Kanagawa, Japan[73] Assignee: **Fuji Photo Film Co., Ltd., Kanagawa, Japan**[21] Appl. No.: **127,091**[22] Filed: **Sep. 27, 1993****Related U.S. Application Data**

[63] Continuation of Ser. No. 836,958, Feb. 19, 1992, abandoned.

[30] **Foreign Application Priority Data**

Feb. 19, 1991 [JP] Japan ..... 3-45459

[51] Int. Cl.<sup>5</sup> ..... G03C 7/42

[52] U.S. Cl. ..... 430/393; 430/455; 430/460

[58] Field of Search ..... 430/393, 455, 460

[56] **References Cited****U.S. PATENT DOCUMENTS**

|           |         |                 |         |
|-----------|---------|-----------------|---------|
| 4,707,434 | 11/1987 | Koboshi et al.  | 430/460 |
| 4,748,105 | 5/1988  | Kadota et al.   | 430/393 |
| 4,908,300 | 3/1990  | Koboshi et al.  | 430/460 |
| 4,983,503 | 1/1991  | Ishikawa et al. | 430/393 |

*Primary Examiner*—Hoa Van Le*Attorney, Agent, or Firm*—Sughrue, Mion, Zinn, Macpeak & Seas[57] **ABSTRACT**

A process and composition for processing a silver halide photographic material. The photographic material may be a black and white photographic material or a color photographic material. The photographic material is processed in a photographic processing bath containing at least one compound represented by the following formula (I) and substantially not containing a thiosulfate ion:



wherein Q represents an atomic group necessary for forming a 5- or 6-membered heterocyclic ring, which heterocyclic ring may be condensed with a carbon aromatic ring or a hetero-aromatic ring; R represents an alkyl group, an alkenyl group, an aralkyl group, an aryl group or a heterocyclic group, each group represented by R being substituted by at least one substituent selected from the group consisting of a carboxyl group or salt thereof or a sulfonic acid group or salt thereof or a phosphonic acid group or salt thereof, an amino group and an ammonium group, or R represents a single bond; n represents an integer or from 1 to 3; and M represents a cation group.

**7 Claims, No Drawings**

**PROCESS OF PROCESSING SILVER HALIDE  
PHOTOGRAPHIC MATERIAL AND  
PHOTOGRAPHIC PROCESSING COMPOSITION  
HAVING A FIXING ABILITY**

This is a continuation of application Ser. No. 07/836,958 filed Feb. 19, 1992, now abandoned.

**FIELD OF THE INVENTION**

The present invention relates to a process for processing a silver halide photographic material, said process providing excellent fixing properties and also excellent stability of a processing bath containing a fixing agent and the bath subsequent thereto, even in the case of low replenishment processing.

The present invention further relates to an improved fixing or blixing composition for fixing or blixing a silver halide photographic material.

**BACKGROUND OF THE INVENTION**

Generally, photographic processing of a silver halide color photographic material comprises a color developing step and a silver removing (desilvering) step. Silver formed by development is oxidized with a 25 bleaching agent and then dissolved with a fixing agent.

A ferric (III) ion complex salt (e.g., an aminopolycarboxylic acid-iron (III) complex salt) is usually used as the bleaching agent and a thiosulfate is usually used as a fixing agent.

Also, processing of a black and white photographic material comprises a development step and a step of removing unexposed silver halide. Unlike processing of a color photographic material, the black and white photographic material is fixed after development without being bleached. In this case, as the fixing agent, a thiosulfate is usually also used.

Recently, with the development of low replenishing techniques, a more stable liquid composition has been desired for each processing bath. As to a fix bath, since the thiosulfate generally contained therein tends to be deteriorated by oxidation, sulfurized and precipitated; a sulfite is usually added to the fix bath as a preservative for preventing the occurrence of the oxidation. However, with the further development of low replenishing techniques, there is yet a further need for improvement of the stability of each processing liquid. However, such improvement is not attained by an increase in the addition amount of sulfite due to the solubility limit of the sulfite. Furthermore, when the sulfite is oxidized, Glau- 50 ber's salt is precipitated.

On the other hand, from the view point of promoting rapid photographic processing, the development of a compound having a fixing property superior to thiosulfate has been desired.

In view of the above, there is a need in the art for the development of a fixing agent having excellent stability to oxidation and an excellent fixing property in place of thiosulfate; however such a compound having the above described properties has not hitherto been known.

**SUMMARY OF THE INVENTION**

A first object of the present invention, therefore, is to provide a fixing process having an excellent fixing property.

A second object of the present invention is to provide a process for processing a silver halide photographic

material having improved stability of a processing bath containing a fixing agent and the bath subsequent thereto under conditions of low replenishment processing.

5 The present inventors have discovered that the foregoing objects can be achieved by the following processing process and processing composition of the present invention.

Namely, in accordance with a first embodiment of the present invention, a process is provided for processing an imagewise exposed silver halide photographic material comprising a support having thereon at least one light-sensitive silver halide emulsion layer, comprising developing in a developing bath and treating in a processing bath having a fixing ability containing at least one compound represented by the following formula (I) as a fixing agent and substantially not containing a thiosulfate ion:

20



wherein Q represents an atomic group necessary for forming a 5- or 6-membered heterocyclic ring, which heterocyclic ring may be condensed with a carbon aromatic ring or a hetero-aromatic ring; R represents an 30 alkyl group, an alkenyl group, an aralkyl group, an aryl group or a heterocyclic group each group represented by R being substituted by at least one substituent selected from the group consisting of a carboxyl group or salt thereof, a sulfonic acid group or salt thereof, a phosphonic acid group or salt thereof, an amino group and an ammonium group, or R represents a single bond (wherein the "single bond" means that the carboxylic group or salt thereof, sulfonic acid group or salt thereof, phosphonic acid group or salt thereof, amino group, or ammonium group is directly bonded to the heterocyclic ring represented by Q); n represents an integer of from 1 to 3; and M represents a cation group.

According to a second embodiment of this invention, there is provided a photographic processing composition having a fixing ability containing at least one compound represented by above-described formula (I) as a fixing agent and substantially not containing a thiosulfate ion.

**DETAILED DESCRIPTION OF THE INVENTION**

The present invention is described in detail below.

First, the compound represented by above-described formula (I) is described in detail.

55 In formula (I), Q preferably represents an atomic group necessary for forming a 5- or 6-membered heterocyclic ring containing carbon and at least one atom selected from a nitrogen atom, an oxygen atom, a sulfur atom and a selenium atom. Furthermore, the heterocyclic ring may be condensed with a carbon aromatic ring or a hetero-aromatic ring.

60 Examples of the heterocyclic ring include a tetrazole ring, triazole ring, imidazole ring, thiadiazole ring, oxadiazole ring, selenadiazole ring, oxazole ring, thiazole ring, benzoxazole ring, benzothiazole ring, benzimidazole ring, pyrimidine ring, triazaindene ring, tetraazaindene ring, and pentaazaindene ring.

In formula (I), R represents an alkyl group having from 1 to 10 carbon atoms (e.g., methyl, ethyl, propyl, butyl, isopropyl, 2-hydroxypropyl, hexyl, and octyl), an alkenyl group having from 2 to 10 carbon atoms (e.g., vinyl, propenyl and butenyl), an aralkyl group having from 7 to 12 carbon atoms (e.g., benzyl and phenethyl), an aryl group having from 6 to 12 carbon atoms (e.g., phenyl, 2-chlorophenyl, 3-methoxyphenyl, and naphthyl), or a heterocyclic group having from 1 to 10 carbon atoms (e.g., pyridyl, thienyl, furyl, triazolyl, and imidazolyl). Each group represented by R is substituted by at least one substituent selected from a carboxyl group or salt thereof (e.g., a sodium salt, a potassium salt, an ammonium salt, and a calcium salt), a sulfonic acid group or salt thereof (e.g., a sodium salt, a potassium salt, an ammonium salt, a magnesium salt, and a calcium salt), a phosphonic acid group or salt thereof (e.g., a sodium salt, potassium salt, and an ammonium salt), a substituted amino group having from 1 to 10 carbon atoms or unsubstituted amino group (e.g., unsubstituted amino, dimethylamino, diethylamino, methylamino, and bismethoxyethylamino), and a substituted ammonium group having 3 to 12 carbon atoms or unsubstituted ammonium group (e.g., trimethylammonium, triethylammonium, and dimethylbenzylammonium), or R represents a single bond.

Also, R may be a group composed of a combination of the above described alkyl group, alkenyl group, aralkyl group, aryl group, and heterocyclic group (e.g., benzyl, phenethyl, styryl and an alkyl group substituted by a heterocyclic ring) or may contain a linking group selected from  $-\text{CO}-$ ,  $-\text{CS}-$ ,  $-\text{SO}_2-$ ,  $-\text{O}-$ ,  $-\text{S}-$  and  $-\text{NR}_1-$  [wherein  $\text{R}_1$  represents a hydrogen atom, an alkyl group having from 1 to 6 carbon atoms (e.g., methyl, ethyl, butyl, and hexyl), an aralkyl group having from 7 to 10 carbon atoms (e.g., benzyl and phenethyl), or an aryl group having from 6 to 10 carbon atoms (e.g., phenyl and 4-methylphenyl) and combinations thereof (e.g.,  $-\text{COO}-$ ,



M represents a cation group (e.g., a hydrogen atom, an alkali metal atom such as sodium, potassium, etc.; an alkaline earth metal such as magnesium, calcium, etc.; and an ammonium group such as ammonium, triethylammonium, etc.).

In formula (I), the heterocyclic group represented by Q and each group represented by R may be substituted by a nitro group, a halogen atom (e.g., chlorine and bromine), a mercapto group, a cyano group, a substituted or unsubstituted alkyl group (e.g., methyl, ethyl, propyl, t-butyl, and cyanoethyl), a substituted or unsubstituted aryl group (e.g., phenyl, 4-methanesulfonamidophenyl, 4-methylphenyl, 3,4-dichlorophenyl, and naphthyl), a substituted or unsubstituted alkenyl group (e.g., allyl group), a substituted or unsubstituted aralkyl group (e.g., benzyl, 4-methylbenzyl, and phenethyl), a substituted or unsubstituted sulfonyl group (e.g., methanesulfonyl, ethanesulfonyl, and p-toluenesulfonyl), a substituted or unsubstituted carbamoyl group (e.g., unsubstituted carbamoyl, methylcar-

bamoyl, and phenylcarbamoyl), a substituted or unsubstituted sulfamoyl group (e.g., unsubstituted sulfamoyl, methylsulfamoyl, and phenylsulfamoyl), a substituted or unsubstituted carbonamido group (e.g., acetamido and benzamido), a substituted or unsubstituted sulfonamido group (e.g., methanesulfonamido, benzenesulfonamido, and p-toluenesulfonamido), a substituted or unsubstituted acyloxy group (e.g., acetoxy and benzoxyloxy), a substituted or unsubstituted sulfonyloxy group (e.g., methanesulfonyloxy), a substituted or unsubstituted ureido group (e.g., unsubstituted ureido group, methylureido, ethylureido, and phenylureido), a substituted or unsubstituted thioureido group (unsubstituted thioureido and methylthioureido), a substituted or unsubstituted acyl group (e.g., acetyl and benzoyl), an oxycarbonylamino group (e.g., methoxycarbonylamino, phenoxy carbonylamino, and 2-ethylhexyloxycarbonylamino), a hydroxy group, etc.

In formula (I), n represents an integer of from 1 to 3 and when n is 2 or 3, each R group may be the same or different.

In above-described formula (I), Q preferably represents a tetrazole ring, triazole ring, imidazole ring, oxadiazole ring, triazaindene ring, tetraazaindene ring, or pentaazaindene ring; R preferably represents an alkyl group having from 1 to 6 carbon atoms substituted by 1 or 2 substituents selected from a carboxyl group acid or salt thereof and sulfonic acid group or salt thereof; and n preferably represents 1 or 2.

Preferred compounds represented by formula (I) are those shown by the following formula (II):



wherein M and R are defined as in formula (I); T and U each represents C—R' or N (wherein R' represents a hydrogen atom, a halogen atom, a hydroxy group, a nitro group, an alkyl group, an alkenyl group, an aralkyl group, an aryl group, a carbonamido group, a sulfonamido group, a ureido group, a thioureido group, or R as defined in formula (I), and when R' represents R, R' and R in formula (II) may be the same or different.

The compound represented by formula (II) is described in detail below.

T and U represent C—R' or N, and R' represents a hydrogen atom, a halogen atom (e.g., chlorine and bromine), a hydroxy group, a nitro group, an alkyl group having preferably 1 to 10 carbon atoms (e.g., methyl, ethyl, methoxyethyl, n-butyl, and 2-ethylhexyl), an alkenyl group having preferably 2 to 10 carbon atoms (e.g., allyl), an aralkyl group having preferably 7 to 15 carbon atoms (e.g., benzyl, 4-methylbenzyl, phenethyl, and 4-methoxybenzyl), an aryl group having preferably 6 to 15 carbon atoms (e.g., phenyl, naphthyl, 4-methanesulfonamidophenyl, and 4-methylphenyl), a carbonamido group having preferably 1 to 10 carbon atoms (e.g., acetylamino, benzylamino, and methoxypropionylamino), a sulfonamido group having preferably 0 to 10 carbon atoms (e.g., methanesulfonamido, benzenesulfonamido, and p-toluenesulfonamido), a ureido group having preferably 1 to 10 carbon atoms (e.g., unsubstituted ureido, methylureido, and phenylureido), a thioureido group having preferably 1

to 10 carbon atoms (e.g., unsubstituted thioureido, methylthioureido, methoxyethylthioureido, and phenylthioureido), or R as defined in formula (I).

When R' represents R, R' may be the same as R in formula (II) or different.

In formula (II), preferably T and U are each N, or T and U are each C—R' (wherein R' represents a hydrogen atom or an alkyl group having from 1 to 4 carbon atoms) and R preferably represents an alkyl group having from 1 to 4 carbon atoms substituted by 1 or 2 substituents selected from a carboxyl group or salt thereof and a sulfonic acid group or salt thereof.

Specific examples of the compound represented by formula (I) or (II) for use in this invention are illustrated below, but the invention is not limited to these compounds.



-continued



-continued



-continued



-continued



The compounds represented by formulae (I) and (II) for use in this invention can be synthesized according to the methods described in *Berichte der Deutschen Chemischen Gesellschaft*, 28, 77 (1895), JP-A-50-37436, JP-A-51-3231 (the term "JP-A" as used therein means an "unexamined published Japanese patent application"), 50 U.S. Pat. Nos. 2,295,976 and 3,376,310, *Berichte der Deutschen Chemischen Gesellschaft*, 22, 568(1889), ibid., 29, 2483(1896), *Journal of Chemical Society*, 1932, 1806, *Journal of the American Chemical Society*, 71, 400(1949), U.S. Pat. Nos. 2,585,388 and 2,541,924, *Advanced in Heterocyclic Chemistry*, 9, 165(1968), *Organic Synthesis*, IV, 569(1963), *Journal of the American Chemical Society*, 45, 2390(1923), *Chemische Berichte*, 9, 465(1876), JP-B-40-28496 (the term "JP-B" as used herein means an "examined published Japanese patent application"), 60 JP-A-50-89034, U.S. Pat. Nos. 3,106,467, 3,420,670, 2,271,229, 3,137,578, 3,148,066, 3,511,663, 3,060,028, 3,271,154, 3,251,691, 3,598,599, and 3,148,066, JP-B-43-4135, U.S. Pat. Nos. 3,615,616, 3,420,664, 3,071,465, 2,444,605, 2,444,606, 2,444,607, and 2,935,404 and also 65 according to the typical synthesis examples shown below.

SYNTHESIS EXAMPLE 1 (SYNTHESIS OF COMPOUND 1)

After adding 100 ml of water to a mixture of 56.8 g of 2-sulfoethyl isocyanate sodium salt and 22.7 g of sodium azide, the resultant mixture was stirred for 4 hours at 70° C. After the reaction was complete, insoluble materials were removed by filtration, the filtrate was evaporated to dryness under reduced pressure, and the solids thus obtained were recrystallized from 400 ml of methanol to provide 45.1 g (yield 64.7%) of the desired product having a melting point of higher than 300° C. The compound obtained was confirmed to be the desired compound (Compound 1) by NMR, mass spectroscopy and elemental analysis.

SYNTHESIS EXAMPLE 2 (SYNTHESIS OF COMPOUND 13)

After adding 230 ml of water to a mixture of 30.0 g of 2-sulfoethyl isothiocyanate sodium salt and 9.6 g of formylhydrazine, the resultant mixture was stirred for 2 hours at room temperature.

Then, 6.3 g of sodium hydroxide was added to the reaction mixture. After refluxing the mixture for 2 hours, 136 ml of concentrated hydrochloric acid was added to the mixture under ice-cooling. The mixture was then evaporated to dryness under reduced pressure, and the solids thus obtained were recrystallized from 50 ml of water to provide 17.6 g (yield 48.2%) of the desired product having a melting point of 269° C. (decomposed).

The compound obtained was confirmed to be the desired compound (Compound 13) by NMR, mass spectroscopy, and elemental analysis.

SYNTHESIS EXAMPLE 3 (SYNTHESIS OF COMPOUND 18)

After adding 100 ml of water to 38.0 g of 2-sulfoethyl isocyanate sodium salt, 26.8 g of aminoacetaldehyde diethylacetal was added dropwise to the mixture under ice-cooling. Thereafter, the mixture was stirred for 3 hours at 60° C. and after adding thereto 40 ml of acetic acid, the resultant mixture was refluxed for 4 hours. After the reaction was completed, the reaction mixture was evaporated to dryness under reduced pressure. The solids obtained were recrystallized from 200 ml of a mixture of methanol and water (3:1 by vol.) to provide 19.0 g (yield 41.2%) of the desired product having a melting point of 274° C. to 275° C.

The compound obtained was confirmed to be desired compound (compound 18) by NMR, mass spectroscopy, and elemental analysis.

The "bath having a fixing ability" for use in this invention includes, for example, a fix bath and a blix bath (bleach-fix bath).

The "photographic processing composition having a fixing ability" for use in this invention includes, for example, a fixing solution used as a fix bath and a blixing solution used as a blix bath.

The compound represented by formula (I) of this invention is contained in a fix bath preferably in an amount of from  $1 \times 10^{-4}$  to 10 mol/liter, more preferably from  $1 \times 10^{-2}$  to 3 mol/liter, and particularly preferably from  $2 \times 10^{-1}$  to 3 mol/liter. Also, the compound represented by formula (I) of this invention is contained in a blix bath in an amount of from  $2 \times 10^{-2}$  to 10 mol/liter, and preferably from  $2 \times 10^{-1}$  to 3 mol/liter.

When the halogen composition of the silver halide emulsion layer in the photographic material for use in this invention comprises silver iodobromide (e.g., the iodide content is not less than 2 mol %, preferably 3 to 15 mol %), the compound represented by formula (I) of this invention is contained in the processing bath in an amount of preferably from 0.5 to 2 mol/liter, and more preferably from 1.2 to 2 mol/liter. When the above-described halogen composition comprises silver bromide, silver chlorobromide or silver halide having a high silver chloride content (e.g., the chloride content is not less than 80 mol %, preferably 90 to 100 mol %, more preferably 95 to 99.5 mol %), the compound represented by formula (I) of this invention is contained in the processing bath in an amount of preferably from  $2 \times 10^{-1}$  to 1 mol/liter.

The term "substantially does not contain a thiosulfate ion" in the composition having a fixing ability of this invention means that the content of the thiosulfate ion (e.g., ammonium thiosulfate) in the composition is less than 0.1 mol/liter more preferably less than 0.05 mol/liter, and particularly preferably less than 0.01 mol/liter. As discussed above, the compound represented by formula (I) of this invention when used in sufficient quantity is alone effective as a fixing agent. In a preferred embodiment, the composition having a fixing ability for use in this invention substantially does not contain any fixing agent other than the compound represented by formula (I). Recently with the development of low replenishment processing in which the replenishment rate is reduced to from  $\frac{1}{2}$  to 1/10 time that of usual processing, it has been desired to improve the liquid stability of each processing bath. The stability of a fix bath (or blix bath) and a subsequent wash bath is adversely affected by the precipitation of a sulfide formed by the oxidative deterioration of a thiosulfate employed as a fixing agent. The problem also occurs in a wash bath subsequent to the fix or blix bath due to carryover into the wash bath. For preventing precipitation, a sulfite is usually used. However, at low replenishment rates, the foregoing problems are not solved by increasing the sulfite content due to the solubility limit of the sulfite and the formation of Glauber's salt precipitate formed by oxidation of the sulfite.

As the result of various investigations of fixing agents having excellent stability to oxidation which might be used in place of a thiosulfate, the present inventors have discovered that the compound represented by formula (I) of this invention has good fixing ability and is stable to oxidation, and furthermore does not form a precipitate at low replenishing rates. On the other hand, in a blix bath, when a thiosulfate is present together with the compound of formula (I), precipitate forms at low replenishing rates in the blix bath and a subsequent wash bath. The precipitate forms because the oxidizing property of the blix solution itself is considerably higher than that of the fixing solution. However, when the only fixing agent contained in the blix solution is a compound of formula (I) of this invention, good liquid stability is obtained without formation of a precipitate.

Furthermore, the addition of the compound represented by formula (I) of this invention to a wash bath or a stabilization bath subsequent to a bath having a fixing ability is also effective for preventing the formation of a precipitate. The concentration of the compound of formula (I) in the wash bath or stabilization bath is preferably from  $10^{-3}$  to 0.5 times that of the fixing agent in the pre-bath thereof i.e., a fix bath or a blix bath.

A silver halide color photographic material and a process for processing the photographic material in accordance with the present invention are described in detail below.

The silver halide color photographic material for processing in accordance with this invention preferably comprises a support having thereon at least one of a blue-sensitive silver halide emulsion layer, a green-sensitive silver halide emulsion layer, and a red-sensitive silver halide emulsion layer. There are no particular restrictions on the number of layers and the arrangement order of the silver halide emulsion layer(s) and light-insensitive layer(s).

A typical example is a silver halide color photographic material comprising a support having thereon on at least one light-sensitive layer comprising plural silver halide emulsion layers each having the same color sensitivity but having a different light-sensitivity. Furthermore, the light-sensitive layer is a unit light-sensitive layer having a color sensitivity to one of blue light, green light, and red light. In a multilayer silver halide color photographic material, such unit light-sensitive layers are generally arranged in the order of a red-sensitive layer, a green-sensitive layer and a blue-sensitive layer, wherein the blue-sensitive layer is arranged farthest from the support. However, depending on the intended application, other arrangement orders of the unit light-sensitive layers can be used. Furthermore, a light-sensitive layer having a different color sensitivity may be arranged between light-sensitive layers having the same color sensitivity.

Also, various light-insensitive layers such as an interlayer, a protective layer, a subbing layer, etc., may be formed between the above described silver halide light-sensitive layers or as the uppermost layer or the lowermost layer of the photographic material.

The interlayer may contain a coupler, DIR compound, etc., as described in JP-A-61-43748, JP-A-59-113438, JP-A-59-113440, JP-A-61-20037, and JP-A-61-20038 or may contain a color mixing inhibitor as generally employed.

As the plural silver halide emulsion layers constituting each unit light-sensitive layer, a two-layer construction of a high-sensitivity silver halide emulsion layer and a low-sensitivity silver halide emulsion layer as described in West German Patent 1,121,470 and British Patent 923,045 is preferably used. Usually, it is preferable to arrange the light-sensitive emulsion layers constituting the unit layer such that the light-sensitivity is successively lowered towards the support. A light-insensitive layer may also be arranged between silver halide emulsion layers. Also, a low-sensitivity emulsion layer may be arranged farther from the support and a high-sensitivity emulsion layer may be arranged closer to the support as described in JP-A-57-112751, JP-A-62-200350, JP-A-62-206541, and JP-A-62-206543.

For example, the light-sensitive silver halide emulsion layers can be arranged in the order of a low-sensitivity blue-sensitive layer (BL)/a high-sensitivity blue-sensitive layer (BH)/a high-sensitivity green-sensitive layer (GH)/a low-sensitivity green-sensitive layer (GL)/a high-sensitivity red-sensitive layer (RH)/a low-sensitivity red-sensitive layer (RL), or in the order of BH/BL/GL/GH/RH/RL, or the order of BH/BL/GH/GL/RL/RH, wherein the last named layer is arranged farthest from the support.

Further, the layers can be arranged in the order, from the side furthest from the support, of blue sensitive

layer/GH/RH/GL/RL as disclosed in JP-B-55-34932. Furthermore, the layers can also be arranged in the order, from the side furthest from the support, of blue sensitive layer/GL/RL/GH/RH as disclosed in JP-A-56-25738 and JP-A-62-63936.

Also, a three-layer unit construction comprising a high light sensitivity silver halide emulsion layer as the uppermost layer, a silver halide emulsion layer having a light sensitivity lower than that of the uppermost layer 10 as an intermediate layer, and a silver halide emulsion layer having a light sensitivity lower than that of the intermediate layer can be used, wherein the light sensitivity of these silver halide emulsion layers become successively lower towards the support as described in JP-B-49-15495. In the case of employing a three-layer unit construction of the same color sensitivity, each layer of which having a different light sensitivity, the silver halide emulsion layers may be arranged in the order of an intermediate light-sensitive emulsion 15 layer/a high light-sensitive emulsion layer/a low light-sensitive emulsion layer, wherein the intermediate light-sensitive emulsion layer is farthest from the support as described in JP-A-59-202464.

As described above, various layer structures and 20 layer arrangement orders can be selected depending on the intended application of the color photographic light-sensitive material.

When the silver halide color photographic material is a color negative photographic film or a color reversal photographic film, the silver halide contained in the photographic emulsion layers is preferably silver iodobromide, silver iodochloride, or silver iodochlorobromide each containing less than about 30 mol % of silver iodide. Silver iodobromide or silver iodochlorobromide 25 each containing from about 2 mol % to about 25 mol % silver iodide is particularly preferred.

When the silver halide color photographic material is a color photographic paper, the silver halide contained in the photographic emulsion layers is preferably silver chlorobromide or silver chloride substantially not containing silver iodide. The term "substantially not containing silver iodide" as used herein means that the content of silver iodide is less than 1 mol %, and preferably less than 0.2 mol %. The silver chlorobromide emulsions is not particularly limited with respect to halogen composition and any ratio of silver bromide/silver chloride can be used. The ratio is selected in a wide range depending on the intended purpose, but a silver chlorobromide emulsion containing at least 2 mol 30 % silver chloride is preferably used.

For a silver halide color photographic material adapted for rapid processing, a high silver chloride emulsion having a high silver chloride content is preferably used. The silver chloride content of the high silver chloride emulsion is preferably at least 90 mol %, and more preferably at least 95 mol %. For reducing the amount of the replenisher for the various processing solutions, an almost pure silver chloride emulsion having a silver chloride content of from 98 mol % to 99.9 mol % is also preferably used.

The silver halide grains in the photographic silver halide emulsion may have a regular crystal form such as cubic, octahedral, tetradecahedral, etc., an irregular form such as spherical, tabular, etc., a form having a crystal defect such as twin planes, etc., or may be a composite form thereof.

The silver halide grains may be fine grains having a grain size of less than about 0.2  $\mu\text{m}$ , or as large as about

10  $\mu\text{m}$  calculated as a diameter of the projected area. Also, the silver halide emulsion may be a polydisperse emulsion or a monodisperse emulsion.

The silver halide photographic emulsion for use in this invention can be prepared using the methods described, e.g., in *Research Disclosure (RD)*, No. 17643 (December, 1978) pages 22 to 23 "Emulsion Preparation and Types" and *ibid.*, No. 18716 (November, 1979), page 648. Also, the monodisperse silver halide emulsions described in U.S. Pat. Nos. 3,574,628 and 3,655,394 and British Patent 1,413,748 are preferably used in this invention.

Also, tabular silver halide grains having an aspect ratio of at least about 5 can be used in this invention. Tabular silver halide grains are readily prepared by the methods described in Gutoff, *Photographic Science and Engineering*, Vol. 14, 248-257(1970), U.S. Pat. Nos. 4,434,226, 4,414,310, 4,433,048, and 4,439,520 and British Patent 2,112,157.

The silver halide grains may have a uniform halogen composition (crystal structure) throughout the grain, or may have a halogen composition that differs between the inside and the surface portion of the grain, or may have a layer structure. Also, the silver halide grains may be epitaxially joined with a silver halide having a different halogen composition or a compound other than silver halide, such as silver rhodanide, lead oxide, etc. Also, a mixture of silver halides each having various crystal forms may be used.

The silver halide emulsion is generally physically ripened, chemically sensitized, and spectrally sensitized prior to use. In the step of physical ripening, various polyvalent metal ion impurities (e.g., salts or complex salts of cadmium, zinc, lead, copper, thallium, iron, ruthenium, rhodium, osmium, palladium, iridium, platinum, etc.) can be introduced into the system.

Examples of the compounds useful for the chemical sensitization are described in JP-A-62-215272, page 18, right under column to page 22, right upper column. Also, additives for use in the above-noted steps are described in *Research Disclosure (RD)*, No. 17643 and RD, No. 18716 and the corresponding portions are summarized in the following table.

Also photographic additives which can be used in this invention are also described in the foregoing two publications (RD), and the corresponding portions thereof are also shown in the table below.

| Additives                                              | RD 17643              | RD 18716                                        |
|--------------------------------------------------------|-----------------------|-------------------------------------------------|
| 1. Chemical Sensitizer                                 | Page 23               | Page 648,<br>right column                       |
| 2. Sensitivity Increasing Agent                        |                       | Page 648,<br>right column                       |
| 3. Spectral Sensitizer and Supersensitizer             | Pages 23 to 24        | Page 648, right column                          |
| 4. Whitening Agent                                     | Page 24               |                                                 |
| 5. Antifogging and Stabilizer                          | Pages 24 to 25        | Page 649,<br>right column                       |
| 6. Light-Absorbent, Filter Dye, Ultra-violet Absorbent | Pages 25 to 26        | Page 649, right column to page 650, left column |
| 7. Stain Inhibitor                                     | Page 25, right column | Page 650, left column to right column           |
| 8. Dye Image Stabilizer                                | Page 25               |                                                 |
| 9. Hardening Agent                                     | Page 26               | Page 651,<br>left column                        |
| 10. Binder                                             | Page 26               | Page 650,<br>right column                       |
| 11. Plasticizer, Lubricant                             | Page 27               | Page 650,<br>right column                       |

-continued

| Additives                             | RD 17643       | RD 18716                   |
|---------------------------------------|----------------|----------------------------|
| 12. Coating Aid, Surface Active Agent | Pages 26 to 27 | Page 650,<br>right column' |
| 13. Static Inhibitor                  | Page 27        | Page 650,<br>right column  |

Also, for preventing the deterioration of photographic performance upon contact with formaldehyde gas, a compound capable of fixing formaldehyde as described in U.S. Pat. Nos. 4,411,987 and 4,435,503 is preferably incorporated into the silver halide color photographic material.

Various color couplers can be contained in the photographic material for processing in accordance with this invention, and practical examples thereof are described in the patents cited in RD, No. 17643, VII-C to G.

Preferred examples of yellow couplers are described in U.S. Pat. Nos. 3,933,501, 4,022,620, 4,326,024, 4,401,752, and 4,248,961, JP-B-58-10739, British Patents 1,425,020 and 1,476,760, U.S. Pat. Nos. 3,973,968, 4,314,023, and 4,511,649 and European Patent 249,473A.

Preferred magenta couplers include 5-pyrazolone series compounds and pyrazoloazole series compounds, and particularly preferred magenta couplers are described in U.S. Pat. Nos. 4,310,619 and 4,351,897, European Patent 73,636, U.S. Pat. Nos. 3,061,432 and 3,725,064, RD, No. 24220 (June, 1984), RD, No. 24230 (June, 1984), JP-A-60-33552, JP-A-60-43659, JP-A-61-72238, JP-A-60-35730, JP-A-55-118034, and JP-A-60-185951, U.S. Pat. Nos. 4,500,630, 4,540,654, and 4,556,630, WO (PCT) 88/04795.

The cyan couplers include phenol series couplers and naphthol series couplers. Preferred examples of the cyan coupler are described in U.S. Pat. Nos. 4,052,212, 4,146,396, 4,228,233, 4,296,200, 2,369,929, 2,801,171, 2,772,162, 2,895,826, 3,772,002, 3,758,308, 4,334,011, and 4,327,173, West German Patent Application (OLS) 3,329,729, European Patents 121,365A and 249,453A, U.S. Pat. Nos. 3,446,622, 4,333,999, 4,753,871, 4,451,559, 4,427,767, 4,690,889, 4,254,212, and 4,296,199 and JP-A-61-42658.

In this invention, a colored coupler for correcting the unnecessary absorption of a colored dye can be used, and preferred examples thereof are described in RD, NO. 17643, VII-G, JP-B-57-39413, U.S. Pat. Nos. 4,163,670, 4,004,929, and 4,138,258, and British Patent 1,146,368.

Also, in this invention, it is preferable to use a coupler for correcting the unnecessary absorption of a colored dye by means of a fluorescent dye released at coupling as described in U.S. Pat. No. 4,774,181 or a coupler having a dye precursor which forms a dye by reacting with a color developing agent as a releasing group as described in U.S. Pat. No. 4,777,120.

In this invention, a coupler forming a colored dye having a proper diffusibility can be used, and preferred examples thereof are described in U.S. Pat. No. 4,366,237, British Patent 2,125,570, European Patent 96,570 and West German Patent Application (OLS) 3,234,533.

Also, in this invention, a polymerized dye-forming coupler can be used, and typical examples thereof are described in U.S. Pat. Nos. 3,451,820, 4,080,211, 4,367,282, 4,409,320, and 4,576,910, and British Patent 2,102,173.

A coupler releasing a photographically useful group upon coupling is preferably used in this invention. Preferred examples of a DIR coupler which releases a development inhibitor are described in the patents cited in RD, 17643, VII-F, JP-A-57-151944, JP-A-57-154234, JP-A-60-184248, and JP-A-63-37346, U.S. Pat. Nos. 4,248,962 and 4,782,012.

Furthermore, in this invention, a coupler which imagewise releases a nucleating agent or a development accelerator upon development can be used, and preferred examples thereof are described in British Patents 2,097,140 and 2,131,188, JP-A-59-157638 and JP-A-59-170840.

Other couplers for use in the silver halide color photographic material in accordance with this invention include competing couplers as described in U.S. Pat. No. 4,130,427, polyequivalent couplers as described in U.S. Pat. Nos. 4,283,472, 4,338,393, and 4,310,618, DIR redox compound-releasing couplers, DIR coupler-releasing couplers, DIR coupler-releasing redox compounds, and DIR redox-releasing redox compounds as described in JP-A-60-185950 and JP-A-62-24252, couplers which release a dye which recolors after being released as described in European Patent 173,302A, bleach accelerator-releasing couplers as described in RD, No. 11449, RD, No. 24241, and JP-A-61-201247, ligand-releasing couplers as described in U.S. Pat. No. 4,553,477, couplers releasing a leuco dye as described in JP-A-63-75747, and couplers releasing a fluorescent dye as described in U.S. Pat. No. 4,774,181.

The couplers for use in this invention can be introduced into the silver halide color photographic material by various dispersion methods.

For example, an oil drop-in-water dispersion method can be employed for this purpose, and examples of high-boiling organic solvents for use in the oil drop-in-water dispersion method are described in U.S. Pat. No. 2,322,027.

Useful examples of the high-boiling organic solvent having a boiling point at atmospheric pressure of at least 175° C. for use in the oil drop-in-water dispersion method include phthalic acid esters (e.g., dibutyl phthalate, dicyclohexyl phthalate, di-2-ethylhexyl phthalate, decyl phthalate, bis(2,4-di-t-amylphenyl phthalate, bis(2,4-di-t-amylphenyl) isophthalate, and bis(1,1-diethylpropyl) phthalate), phosphoric acid esters or phosphonic acid esters (e.g., triphenyl phosphate, tricresyl phosphate, 2-ethyl-hexyldiphenyl phosphate, tricyclohexyl phosphate, 2-tri-2-ethylhexyl phosphate, tridodecyl phosphate, tributoxyethyl phosphate, trichloropropyl phosphate, and di-2-ethylhexylphenyl phosphonate), benzoic acid esters (e.g., 2-ethylhexyl benzoate, dodecyl benzoate, and 2-ethylhexyl-p-hydroxy benzoate), amides (e.g., N,N-diethyldodecanamide, N,N-diethylaurylamide, and N-tetradecylpyrrolidone), alcohols or phenols (e.g., isostearyl alcohol and 2,4-di-tert-amylphenol), aliphatic carboxylic acid esters (e.g., bis(2-ethylhexyl) sebacate, dioctyl azelate, glycerol tributylate, isostearyl lactate, and trioctyl citrate), aniline derivatives (e.g., N,N-dibutyl-2-butoxy-5-tert-octylaniline), and hydrocarbons (e.g., paraffin, dodecylbenzene, and diisopropylnaphthalene).

Also, as an auxiliary solvent, an organic solvent having a boiling point of at least 30° C., and preferably from about 50° C. to about 160° C. can be used. Typical examples of the auxiliary solvent include ethyl acetate, ethyl propionate, methyl ethyl ketone, cyclohexanone, 2-ethoxyethyl acetate, and dimethylformamide.

Also, a latex dispersion method can be employed for introducing the couplers, and practical examples of the involved steps and effects of the latex dispersion method and useful examples of a latex for impregnation are described in U.S. Pat. No. 4,199,363, West German Patent Applications (OLS) 2,541,274 and 2,541,230.

Moreover, the above described couplers can be emulsion-dispersed in an aqueous solution of a hydrophilic colloid by impregnating a loadable latex polymer (as described, e.g., in U.S. Pat. No. 4,203,716) with the coupler in the presence or absence of the above described high-boiling organic solvent or by dissolving the coupler in a polymer which is insoluble in water but soluble in an organic solvent.

Preferred polymers for use with a coupler include the homopolymers or copolymers described in WO 88/00723, pages 12 to 30. In particular, the use of an acrylamide series polymer is preferred with respect to color image stability, etc.

The process of this invention can be applied to various color photographic materials. Typical examples thereof are general or motion picture color negative photographic films, color reversal photographic films for slide or television, color photographic papers, direct positive color photographic materials, color positive photographic films, and color reversal photographic papers.

Supports for use in the photographic material of this invention are described in RD, No. 17643, page 28 and RD, No. 18716, page 647, right column to page 648, left column.

In the silver halide color photographic material for processing in accordance with this invention, the total thickness of the all of the hydrophilic colloid layers on the side having the silver halide emulsion layers is not more than 25  $\mu$ m, and preferably is not more than 20  $\mu$ m. The layer swelling speed  $T_{\frac{1}{2}}$  is preferably not higher than 30 seconds, and preferably not higher than 15 seconds.

Herein, the layer thickness is measured at 25° C. after storing for 2 days in a controlled environment having a relative humidity of 55%. Also, the layer swelling speed  $T_{\frac{1}{2}}$  can be measured by a method known in this field of art. For example, the swelling speed can be measured by using a swellometer of the type described in A. Green et al, *Photographic Science and Engineering*, Vol. 19, No. 2, pages 124-129.  $T_{\frac{1}{2}}$  is defined as the time required to reach a saturated layer thickness which is 90% of the maximum swelled layer thickness attained when processing the color photographic material with a color developer for 3 minutes and 15 seconds at 30° C.

The layer swelling speed  $T_{\frac{1}{2}}$  can be controlled by adding a hardening agent to a binder such as gelatin, or by controlling the storage condition after coating. Also, the swelling ratio is preferably from 150% to 400%. The swelling ratio can be calculated from the maximum swelled layer thickness attained under the condition described above according to the following equation:

$$\text{Swelling ratio} = (A - B)/B$$

A: The maximum swelled layer thickness

B: Layer thickness

The silver halide color photographic material for use in this invention can be developed by the process described in RD, No. 17643, pages 28-29 and RD, No. 18716, page 615, left column to right column.

The color developer for use in developing the color photographic material is preferably an alkaline aqueous solution containing an aromatic primary amine color developing agent as a main component. As the color developing agent, an aminophenol series compound is useful but a p-phenylenediamine series compound is preferably used. Typical examples thereof are 3-methyl-4-amino-N,N-diethylaniline, 3-methyl-4-amino-N-ethyl-N-β-hydroxyethylaniline, 3-methyl-4-amino-N-ethyl-N-β-methanesulfonamidoethylaniline, 3-methyl-4-amino-N-ethyl-β-methoxyethylaniline and the sulfates, hydrochlorides and p-tolyenesulfonates of these compounds. The developing agents can be used alone or in combination thereof.

The color developer generally contains a pH buffer such as a carbonate, borate, or phosphate of an alkali metal, and a development inhibitor or an antifoggant such as a bromide, iodide, benzimidazole, benzothiazole, and mercapto compound. Also, if necessary, the color developer may further contain a preservative such as hydroxylamine, diethylhydroxylamine, sulfite, hydrazines, phenylsemicarbazides, triethanolamine, catecholsulfonic acid, triethylenediamine(1,4-diazabicyclo[2.2.2]octanes); an organic solvent such as ethylene glycol, diethylene glycol, etc.; a development accelerator such as benzyl alcohol, polyethylene glycol, quaternary ammonium salts, amines, etc.; a dye-forming coupler; a competing coupler; a fogging agent such as sodium boron hydride, etc.; an auxiliary developing agent such as 1-pheyl-3-pyrazolidone, etc.; a tackifier; a chelating agent such as an aminopolycarboxylic acid, an aminopolyphosphonic acid, an alkylphosphonic acid, and a phosphonocarboxylic acid [e.g., ethylenediaminetetraacetic acid, nitrilotriacetic acid, diethylenetriaminepentaacetic acid, cyclohexanediaminetetraacetic acid, hydroxyethyliminodiacetic acid, 1-hydroxyethylidene-1,1-diphosphonic acid, nitrilo-N,N,N,N-tetramethylenephosphonic acid, ethylenediamine-N,N,N,N-tetramethylenephosphonic acid, ethylenediaminedi(o-hydroxyphenylacetic acid) and the salts thereof]; a fluorescent whitening agent such as a 4,4'-diamino-2,2'-disulfostilbene series compound, etc.; and a surface active agent such as an alkylsulfonic acid, an arylsulfonic acid, an aliphatic carboxylic acid, an aromatic carboxylic acid, etc.

In the present invention, it is preferable that the color developer contain substantially no benzyl alcohol in view of environmental considerations, liquid preparing properties and color stain inhibition. The term "contains substantially no benzyl alcohol" means that the color developer contains not more than 2 ml of benzyl alcohol per liter of the color developer (more preferably, the color developer contains no benzyl alcohol).

Also, in the case of practicing reversal processing, color development is usually carried out after carrying out black and white development. The black and white developer can contain a known black and white developing agent such as a dihydroxybenzene (e.g., hydroquinone, etc.), a 3-pyrazolidone (e.g., 1-phenyl-3-pyrazolidone), and an aminophenol (e.g., N-methyl-p-aminophenol) used alone or in combination thereof.

The pH of the color developer and the black and white developer is generally from 9 to 12. Also, the amount of the replenisher for the developer is generally not more than 3 liters per m<sup>2</sup> of the light-sensitive photographic material being processed. However, the replenishment rate varies depending on the type of color photographic material. The replenisher amount can be

reduced to below 500 ml/m<sup>2</sup> by reducing the bromide ion concentration in the replenisher. In particular, when using a high silver chloride type color photographic material, it is particularly preferred to reduce bromide ion and to relatively increase chloride ion concentration in the color developer. In this case, the photographic properties and the processing properties are excellent and the variation in photographic properties is readily controlled. The amount of the replenisher for the color developer can then be reduced to about 20 ml/m<sup>2</sup> of the color photographic light-sensitive material being developed. When using such a small amount of replenisher, overflow from the color developing bath does not substantially occur.

When using a low replenishing amount, it is preferable to prevent the evaporation and air-oxidation of the processing solution by reducing the contact area of the processing solution with air. Also, by restricting the accumulation of bromide ion in the developer, the amount of the developer replenisher can be reduced.

The processing temperature of the color developer for use in this invention is from 20° C. to 50° C., and preferably from 30° C. to 45° C. The processing time is from 20 seconds to 5 minutes, and preferably from 30 seconds to 3 minutes. By increasing the processing temperature and pH of the developer and by using a color developer containing a developing agent in high concentration, the processing time can be further reduced.

The photographic emulsion layers are generally bleached after color development. The bleach process may be carried out simultaneously with a fix process (bleach-fix or blix) or may be carried out separately from the fix process. Furthermore, for increasing the processing speed, a blix processing may be carried out after bleach processing. Moreover, a process of processing in a second blix bath immediately following a first blix bath, a process of fixing before blix processing, or a process of bleaching after blix processing can be practiced according to the intended purpose.

The processing temperature of the bleach solution and blix solution is from 20° C. to 50° C., and preferably from 30° C. to 45° C. The processing time is from 20 seconds to 5 minutes, and preferably from 30 seconds to 4 minutes.

As bleaching agents, for example, compounds of a multivalent metal such as iron(III), cobalt(III), chromium(IV), copper(II), etc., peracids, quinones, and nitro compounds can be used.

Useful examples of the bleaching agent include ferricyanides; bichromates; organic complex salts of iron(III) or cobalt(III), such as, for example, the complex salts of aminopolycarboxylic acids such as ethylenediaminetetraacetic acid, diethylenetriaminopentaacetic acid, cyclohexanediaminetetraacetic acid, methylinodiacetic acid, 1,3-diaminopropanetetraacetic acid, glycol ether diaminetetraacetic acid, etc., or citric acid, tartaric acid, malic acid, etc.; persulfates; bromate; permanganates; nitrobenzenes, etc.

Of these bleaching agents, the aminopolycarboxylic acid iron(III) complex salts such as an ethylenediaminetetraacetic acid iron(III) complex salt, etc., and persulfates are preferred for rapid processing and in view of environmental factors. Furthermore, the aminopolycarboxylic acid iron(III) complex salts are particularly useful in both a bleach solution and a blix solution. In particular, in a bleach solution for processing a color photographic negative film for in camera use, 1,3-diaminopropanetetraacetic acid iron(III) complex salts

are preferred in view of their bleaching ability. The pH of the bleach solution or the blix solution containing an aminopolycarboxylic acid iron(III) complex salt is generally from 5.5 to 8, but the processing solution may have lower pH to speed up processing process. The amount of the bleaching agent to be added to the bleach solution or blix solution is preferably from 0.05 to 1 mol/liter.

For the bleach solution, the blix solution and the pre-bath thereof, if necessary, a bleach accelerator can be added thereto.

Examples of useful bleach accelerators are the compounds having a mercapto group or a disulfide group described in U.S. Pat. No. 3,893,858, West German Patents 1,290,812 and 2,059,988, JP-A-53-32736, JP-A-53-57831, JP-A-53-37418, JP-A-53-72623, JP-A-53-95630, JP-A-53-95631, JP-A-53-104232, JP-A-53-124424, JP-A-53-141623, JP-A-53-28426, RD, No. 17129 (July, 1978), etc.; the thiazolidine derivatives described in JP-A-50-140129; the thiourea derivatives described in JP-B-45-8506, JP-A-52-20832, JP-A-53-32735, U.S. Pat. No. 3,706,561, etc.; the iodides described in West German Patent 1,127,715, JP-A-58-16235, etc.; the polyoxyethylene compounds described in West German Patents 966,410 2,748,430, etc.; the polyamine compounds described in JP-B-45-8836, etc.; the compounds described in JP-A-49-42434, JP-A-49-59644, JP-A-53-94927, JP-A-54-35727, JP-A-55-26506, JP-A-58-163940, etc.; and bromide ion.

Of these bleach accelerators, the compounds having a mercapto group or a disulfide group are preferred for providing a large accelerating effect, and the compounds described in U.S. Pat. No. 3,893,858, West German Patent 1,290,812, and JP-A-53-95630 are particularly preferred. Further, the compounds described in U.S. Pat. No. 4,552,834 are also preferred. The amount of the bleach accelerators to be added to the bleach solution or blix solution is preferably  $1 \times 10^{-4}$  to  $1 \times 10^{-2}$  mol/liter, more preferably  $1 \times 10^{-4}$  to  $1 \times 10^{-3}$  mol/liter. The bleach accelerators may also be added to the color photographic light-sensitive material. In the case blixing a color photographic material for in camera use, the above described bleach accelerators are particularly effective.

The blix solution for use in this invention can contain known additives, e.g., a rehalogenating agent such as ammonium bromide, ammonium chloride, etc., a pH buffer such as ammonium nitrate, etc., and a metal corrosion inhibitor such as ammonium sulfate, etc.

The fix bath of this invention may contain a known fixing agent other than a thiosulfate ion in addition to the compound represented by formula (I).

Examples of known fixing agents for use in this invention include thiocyanates, thioether series compounds, thioureas, and iodide in large quantity. The amount of the known fixing agents is approximately the same as that of the compound represented by formula (I). The known fixing agents may be used in any ratio with the compound represented by formula (I).

The blix solution of this invention may contain a preservative such as a sulfite, a bisulfite, a carbonyl-bisulfite addition product, and a sulfonic acid compound.

Also, the fix solution of this invention preferably contains an aminopolycarboxylic acid or an organic phosphonic acid series chelating agent (such as, preferably, 1-hydroxyethylidene-1,1-diphosphonic acid and

N,N,N',N'-ethylenediaminetetraphosphonic acid) for improving the stability of the fix solution.

The processing temperature of the fix solution is from 20° C. to 50° C., and preferably from 30° C. to 45° C.

5 The processing time is from 20 seconds to 5 minutes, and preferably from 30 seconds to 4 minutes.

The fix solution can further contain various fluorescent whitening agents, defoaming agents, surface active agents, polyvinylpyrrolidone, methanol, etc.

10 For shortening the desilvering processing time, vigorous stirring of each processing solution in the desilvering step is preferably carried out. Useful stirring means include the methods described in JP-A-62-183460 and JP-A-62-183461. In the case of applying a

15 jet stream as the stirring means, the jet stream is preferably applied within 15 seconds after introducing the color photographic material into the processing solution.

In this invention, the crossover time from a color

20 developer to a bleach solution (i.e., the time that it takes for a color photographic material to leave the color developer and enter the bleach solution) is preferably 10 seconds or less for improving the bleach fog and to minimize staining of the surface of the color photographic material being processed. Also, the crossover time from the bleach solution to the processing solution

25 having a fixing ability in this invention is preferably 10 seconds or less for improving the inferior recoloring of cyan dyes.

30 The replenishing amount for the fix solution is preferably from 300 to 800 ml/m<sup>2</sup> in the case of a color photographic light-sensitive material for in camera use (e.g., coated silver amount of from 4 to 12 g/m<sup>2</sup>), and the replenishing amount for the blix solution is preferably from 20 to 50 ml/m<sup>2</sup>.

The silver halide color photographic material for processing in accordance with this invention is generally subjected to a wash step and/or a stabilization step after desilvering processing.

40 The amount of wash water in the wash step can be selected in a wide range depending on the characteristics (e.g., materials being used, such as couplers, etc.) of the color photographic material being processed, the use thereof, the temperature of the wash water, the

45 number of wash tanks (stage numbers), the replenishing system such as a counter-current system, a regular current system, etc., and other various conditions. Among these conditions, the relationship of the number of wash tanks and the amount of wash water in a multistage

50 counter-current system can be obtained by the method described in *Journal of the Society of Motion Picture and Television Engineering*, Vol. 64, 248-253 (May, 1955).

In accordance with the multistage counter-current system described in the above publication, the amount

55 of wash water can be greatly reduced. However, the increase in residence time of water in the tanks results in the proliferation of bacteria which float and adhere to the color photographic material. In the processing of a color photographic material in accordance with this

60 invention, effective means for solving the foregoing problems include a method of reducing Ca ion and Mg ion as described in JP-A-62-288838. Chlorine series germicides such as the isothiazolone compounds described in JP-A-57-8542, thiabendazole, chlorinated

65 sodium isocyanurate, etc., other benzotriazoles, and other germicides described in Hiroshi Horiguchi, *Boo-kin Boobai no Kagaku (Chemistry of Antibacterial and Antifungal Agents)*, *Biseibutsu no Mekkin, Sakkin, Boo-*

bai Gijutsu (Germicidal and Fungicidal Techniques of Microorganisms), edited by Eiseigijutsu Kai, and Bookin Boobaizai Jiten (Handbook of Germicidal and Fungicidal Agents), edited by Nippon Bookin Boobai Gakkai can also be used in this invention.

The pH of wash water in the processing of a color photographic material in accordance with this invention is from 4 to 9, and preferably from 5 to 8. The temperature and the time of water washing is selected depending on the characteristics and the use of the color photographic material being processed, but is generally in the range of from 15° C. to 45° C. and from 20 seconds to 10 minutes, and preferably from 25° C. to 40° C. and from 30 seconds to 5 minutes. Furthermore, in the process of this invention, a stabilization step can be directly applied in place of the above noted wash step. For the stabilization step, all of the processes described in JP-A-57-8543, JP-A-58-14834, and JP-A-60-220345 can be used.

In some circumstances, the stabilization process may be further conducted after the wash processing. For example, a stabilization bath containing a dye stabilizer such as formalin, hexamethylenetetramine, hexahydrotetrazine, and an N-methylol compound can be used as a final bath for processing of color photographic materials for in camera use. If necessary, the stabilization bath can contain ammonium compounds, metal compounds of Bi, Al, etc., fluorescent whitening agents, various chelating agents, film pH controlling agents, a hardening agent, germicides, fungicides, alkanoiamine, and surface active agents (preferably silicone series surfactants).

As the water for use in the wash step and the stabilization step, city water, water subjected to a deionizing treatment by an ion exchange resin to reduce the Ca ion concentration and the Mg ion concentration below 5 mg/liter, or water sterilized by a halogen or a ultraviolet sterilizing lamp is preferably used.

The replenishing amount for the above described wash step and/or the stabilization step is from 1 to 50 times, preferably from 2 to 30 times, and more preferably from 2 to 15 times the amount of the processing solution carried over from the pre-bath per unit area of the color photographic material being processed. The overflow liquid obtained with replenishing can be reused for the desilvering step and other steps.

The silver halide color photographic material for processing in accordance with this invention may contain a color developing agent to simplify and accelerate the processing. When contained in the color photographic material, a precursor of the color developing agent is preferably used. For example, useful developing agent precursors include the indoaniline type compounds described in U.S. Pat. No. 3,342,597, the Schiff base type compounds described in U.S. Pat. No. 3,342,599, RD, No. 14850, and RD, No. 15159, the metal complexes described in U.S. Pat. No. 3,719,492, and the urethane series compounds described in JP-A-53-135628.

The silver halide color photographic material for processing in accordance with this invention may contain various 1-phenyl-3-pyrazolidones for accelerating the color development. Typical compounds are described in JP-A-56-64339, JP-A-57-144547, and JP-A-58-115438.

The various processing solutions in this invention are generally used at a temperature of from 10° C. to 50° C. A temperature of from 33° C. to 38° C. is generally

employed, but the processing time can be shortened by employing a higher temperature. On the other hand, improvement of image quality and improvement of the stability of the processing solutions can be attained by employing a lower processing temperature.

An example of a silver halide color photographic material for use in this invention is a direct positive silver halide color photographic material. A process for processing a direct positive silver halide color photographic material in accordance with this invention is described below.

After imagewise exposure of the silver halide color photographic material, direct positive color images are formed preferably by color developing with a surface developer containing an aromatic primary amine color developing agent having pH of not higher than 11.5. The photographic material is subjected to a fogging treatment during or following color development with light or a nucleating agent, and the fogging treatment is followed by bleaching and fixing. The pH of the surface developer is preferably in the range of from 11.0 to 10.0.

For the fogging treatment in accordance with this invention, a "light fogging method" (i.e., a method of applying a secondary exposure to the whole surface of the light-sensitive emulsion layers) or a "chemical fogging method" (i.e., a method of developing in the presence of a nucleating agent) may be used. Furthermore, the color photographic material may be developed in the presence of a nucleating agent and fogging light. Also, the color photographic material containing a nucleating agent may be subjected to a fogging exposure.

The light fogging method is described in Japanese Patent Application No. 61-253716, page 47, line 4 to page 49, line 5 and a nucleating agent which can be used in this invention is described in the same patent application, page 49, line 6 to page 67, line 2. In particular, the use of the compounds shown by general formulae (N-1) and (N-2) described in Japanese Patent Application No. 61-253716 is preferred. Specific examples of the preferred nucleating agent are (N-I-1) to (N-I-10) described in the above noted patent application, page 56 to page 58, and (N-II-1) to (N-II-12) described at pages 63 to 66.

Nucleation accelerators for use in this invention are described in the foregoing Japanese Patent Application No. 61-253716, page 68, line 11 to page 71, line 3. The nucleation accelerators (A-1) to (A-13) described in the above noted patent application, pages 69 to 70, are particularly preferred.

A silver halide black and white photographic material and method for processing thereof in accordance with this invention are described below.

There is no particular restriction on the halogen composition of the light-sensitive silver halide emulsion. Silver chloride, silver chlorobromide, silver iodobromide, silver bromide, silver iodobromochloride, etc., can be used, but the silver iodide content is preferably not more than 10 mol %, and particularly preferably not more than 5 mol %.

For the formation of a negative image having high contrast, the mean grain size of the silver halide grains is preferably not larger than 0.7  $\mu\text{m}$ , and is particularly preferably not larger than 0.5  $\mu\text{m}$ .

There is no particular restriction with respect to grain size distribution of the silver halide grains, but a monodisperse silver halide emulsion is preferred.

The term "monodisperse" means that at least 95% by weight or grain number of the silver halide grains have grain sizes within  $\pm 40\%$  of the mean grain size.

The silver halide grains of the silver halide photographic emulsion may have a regular crystal form such as cubic, octahedral, rhombic dodecahedral, tetradecahedral, etc., an irregular crystal form such as spherical, tabular, etc., or a composite form of these crystal forms.

With regard to other aspects of the silver halide photographic emulsion, the above description regarding silver halide photographic emulsions for use in a photographic material are generally applicable.

The silver halide emulsion layer of a photographic material for use in this invention preferably contains two kinds of monodisperse silver halide emulsions each having a different mean grain size as described in JP-A-61-223734 and JP-A-62-90646 for the purpose of increasing the maximum density (D<sub>max</sub>). In this case, the monodisperse silver halide grains having a smaller grain size is preferably chemically sensitized. Sulfur sensitization is most preferred. The monodisperse silver halide emulsion having a larger grain size may or may not be chemically sensitized. The large grain size monodisperse silver halide emulsion is generally not subjected to chemical sensitization; otherwise black pepper tends to occur. Thus, if the larger grain size monodisperse silver halide emulsion is to be chemically sensitized, a low degree of chemical sensitization is preferred to the extent that black pepper is not formed. In this case, the low degree of chemical sensitization is conducted by the means that the time of subjecting the emulsion to chemical sensitization is shortened as compared with the chemical sensitization for the small grain size monodisperse silver halide emulsion, the temperature during chemical sensitization is lowered as compared to that for the smaller grain monodisperse emulsion, or a reduced amount of chemical sensitizing agent is added.

There is no particular restriction on the sensitivity difference of the larger size monodisperse emulsion and the smaller size monodisperse emulsion, but the sensitivity difference is from 0.1 to 1.0, and preferably from 0.2 to 0.7 as Alog E. Preferably, the larger size monodisperse emulsion has a higher sensitivity. The mean grain size of the smaller size monodisperse silver halide grains is less than about 90%, and preferably less than about 80% of the mean grain size of the larger size monodisperse silver halide grains.

In a light-sensitive material for printing for use in this invention, an image having a super high contrast can be formed by incorporating a nucleating agent into the photographic emulsion layer or other hydrophilic colloid layer. Examples of useful nucleating agents include those described in RD, No. 23516 (November, 1983), page 346 and the various literature cited therein.

Compounds effective for use as a development accelerator or as an accelerator for a nucleating agent for development for use in this invention include the compounds disclosed in JP-A-53-77616, JP-A-54-37732, JP-A-53-137133, JP-A-60-140340, and JP-A-60-14959, and various compounds containing N or S.

The direct positive photographic light-sensitive material for use in this invention may contain a desensitizer in the photographic silver halide emulsion layer(s) and other hydrophilic colloid layers. The organic desensitizer for use in this invention is defined by the polarographic half wave potential, namely, the oxidation reduction potential determined by polarography, wherein the sum of the polaro anodic potential and the cathodic potential becomes positive.

As the organic desensitizer, the compounds shown by general formulae (III) to (V) described in Japanese Patent Application No. 61-280998, pages 55 to 72 are preferably used.

5 The developer for developing the silver halide black and white photographic material in accordance with this invention can contain generally employed additives (e.g., a developing agent, an alkali agent, a pH buffer, a preservative, and a chelating agent). For processing in 10 accordance with this invention, known processes can be used. Furthermore, the processing solutions of this invention may contain known additives generally employed in black and white developers. The processing 15 temperature is generally selected in the range of from 18° C. to 50° C. but a temperature lower than 18° C. or a temperature higher than 50° C. may be employed. The processing time is from 10 seconds to 3 minutes, and preferably from 10 seconds to 1 minute.

20 For the black and white developer, known developing agents such as dihydroxybenzenes (e.g., hydroquinone), 1-phenyl-3-pyrazolidones, aminophenols (e.g., N-methyl-p-aminophenol), etc., can be used alone or in combination thereof.

25 The dihydroxybenzene series developing agent is preferably used in an amount of from 0.05 mol/liter to 0.8 mol/liter. Also, in the case of using a combination of a dihydroxybenzene and a 1-phenyl-3-pyrazolidone or a p-aminophenol, it is preferred that the former is used in 30 an amount of 0.05 mol/liter to 0.5 mol/liter and the latter is used in an amount of not more than 0.06 mol/liter.

35 Sulfite preservatives for use in this invention include sodium sulfite, potassium sulfite, lithium sulfite, sodium bisulfite, potassium metabisulfite and formaldehyde sodium bisulfite.

40 For the black and white developer, and especially a developer for graphic art, a sulfite is added in an amount of at least 0.3 mol/liter. However, if the sulfite content is too high, the sulfite precipitates in the developer to cause a liquid stain. Hence, sulfite is preferably contained in an amount of not more than 1.2 mol/liter.

45 The alkali agent contained in the developer for use in this invention includes pH controlling agents and buffers such as sodium hydroxide, potassium hydroxide, sodium carbonate, potassium carbonate, sodium tertiary phosphate, potassium tertiary phosphate, sodium silicate, potassium silicate, etc.

50 Also, other useful additives contained in the black and white developer include development inhibitors such as boric acid, borax, sodium bromide, potassium bromide, potassium iodide, etc.; organic solvents such as ethylene glycol, diethylene glycol, triethylene glycol, dimethylformamide, methylcellosolve, hexylene glycol, ethanol, methanol, etc.; antifogging agents or black pepper inhibitors such as mercapto series compounds (e.g., 1-phenyl-5-mercaptopentetrazole and sodium 2-mercaptopbenzimidazole), indazole series compounds (e.g., 5-nitroindazole), benzimidazole series compounds (e.g., 5-methylbenzimidazole), etc., and further if necessary, the developer may contain a toning agent, a surface active agent, a defoaming agent, a water softener, a hardening agent, etc. Also, as a silver stain inhibitor, the compounds described in JP-A-56-24347 can be used. Also,

55 to prevent uneven development, the compounds described in JP-A-62-212651 can be used. Furthermore, as a dissolution aid, the compounds described in Japanese Patent Application No. 60-109743 can be used.

The developer for use in this invention can contain boric acid as described in JP-A-62-186259, saccharide (e.g., saccharose), oximes (e.g., acetoxime), phenols (e.g., 5-sulfosalicylic acid), and tertiary phosphates (e.g., the sodium salts and potassium salts) as described in JP-A-60-93433.

The fix solution for use in this invention is an aqueous solution containing, if necessary, a hardening agent (e.g., water-soluble aluminum compounds), acetic acid, and a dibasic acid (e.g., tartaric acid, citric acid and the salts thereof) in addition to the fixing agent. The fix solution preferably has a pH of higher than 3.8, and is preferably from 4.0 to 7.5.

A water-soluble aluminum compound can be used in the fix solution as a hardening agent to provide an acidic hardening fix solution. Examples thereof include aluminum chloride, aluminum sulfate, and aluminum alum.

Also, as the foregoing dibasic acid, tartaric acid or derivatives thereof and citric acid or derivatives thereof can be used alone or in combination thereof. The effective amount of the compound is at least 0.005 mol per liter of the fix solution, and particularly from 0.01 mol/liter to 0.03 mol/liter. Useful examples thereof include tartaric acid, potassium tartarate, sodium tartarate, sodium potassium tartarate, ammonium tartarate, and 25 potassium ammonium tartarate.

If necessary, the fix solution may further contain a preservative (e.g., sulfite and hydrogensulfite), a pH buffer (e.g., acetic acid and boric acid), a pH controlling agent (e.g., ammonia and sulfuric acid), an image storage improving agent (e.g., potassium iodide), and a chelating agent.

In this case, the pH buffer is used in an amount of from 10 g/liter to 40 g/liter, and more preferably from about 18 g/liter to 25 g/liter because the pH of the developer is relatively high.

The fixing temperature and time are the same as those for the development and are preferably from about 20° C. to about 50° C. and from 10 seconds to 1 minute. The replenishing amount for the fix solution is preferably 40 from 50 to 300 ml/m<sup>2</sup>.

Also, the above described wash water for processing can be used. Also, a stabilization solution may be used in place of wash water.

In this invention, the roller transporting type automatic processor described in U.S. Pat. Nos. 3,025,779 and 3,545,971 can be used. The processor is simply referred to herein as a roller transport type processor.

The roller transport type processor is composed of 4 steps of development, fix, wash, and drying. It is most 50 preferable that the processing employ these 4 steps, although other steps (e.g., a stop step) are not excluded. In this case, in the wash step, water consumption can be reduced by using a counter-current wash step of from 2 to 3 stages.

The black and white photographic light-sensitive material for processing in accordance with this invention include an ordinary black and white silver halide photographic material (e.g., black and white photographic paper for in camera use, an X-ray black and white photographic material, and a printing black and white light-sensitive material), an infrared photographic light-sensitive material for laser scanner, etc.

Use of the compound of formula (I) of this invention improves stability (in particular, sulfurization, etc., is 65 prevented) of a fix solution or a fix solution having a bleaching ability (e.g., a blix solution), and a processing composition having a good fixing ability is obtained.

Also, by using the compound of formula (I) of this invention, stable processing is achieved even when the replenishing amount for the fix solution or the blix solution is greatly reduced.

The invention is further described in reference to the following Examples, but the invention is not limited thereby.

#### EXAMPLE 1

A multilayer color photographic material (sample 101) was prepared by forming the layers having the following compositions on a cellulose triacetate film support having a subbing layer. (Compositions of Layers)

The coating amounts are shown in terms of the unit g/m<sup>2</sup> of silver for a silver halide emulsion and colloidal silver, the unit g/m<sup>2</sup> for couplers, additives and gelatin, and the unit mol number per mol of the silver halide contained in the same layer for a sensitizing dye.

| <u>Layer 1 (Antihalation Layer)</u>                                                                                                                                                                                                 |                      |
|-------------------------------------------------------------------------------------------------------------------------------------------------------------------------------------------------------------------------------------|----------------------|
| Black Colloidal Silver                                                                                                                                                                                                              | 0.15                 |
| Gelatin                                                                                                                                                                                                                             | 1.5                  |
| ExM-8                                                                                                                                                                                                                               | 0.08                 |
| UV-1                                                                                                                                                                                                                                | 0.03                 |
| UV-2                                                                                                                                                                                                                                | 0.06                 |
| Solv-2                                                                                                                                                                                                                              | 0.08                 |
| UV-3                                                                                                                                                                                                                                | 0.07                 |
| Cpd-5                                                                                                                                                                                                                               | $6 \times 10^{-4}$   |
| <u>Layer 2 (Interlayer)</u>                                                                                                                                                                                                         |                      |
| Gelatin                                                                                                                                                                                                                             | 1.5                  |
| UV-1                                                                                                                                                                                                                                | 0.03                 |
| UV-2                                                                                                                                                                                                                                | 0.06                 |
| UV-3                                                                                                                                                                                                                                | 0.07                 |
| ExF-1                                                                                                                                                                                                                               | 0.004                |
| Solv-2                                                                                                                                                                                                                              | 0.07                 |
| Cpd-5                                                                                                                                                                                                                               | $6 \times 10^{-4}$   |
| <u>Layer 3 (1st Red-Sensitive Emulsion Layer)</u>                                                                                                                                                                                   |                      |
| Silver Iodobromide Emulsion (AgI 2 mol %, high internal AgI type, sphere-corresponding diameter 0.3 $\mu$ m, variation coeff. of sphere-corresponding diameter 29%, normal crystal and twin crystal mixed grains, aspect ratio 2.5) | 0.5                  |
| Gelatin                                                                                                                                                                                                                             | 0.8                  |
| ExS-1                                                                                                                                                                                                                               | $1.0 \times 10^{-4}$ |
| ExS-2                                                                                                                                                                                                                               | $3.0 \times 10^{-4}$ |
| ExS-3                                                                                                                                                                                                                               | $1 \times 10^{-5}$   |
| ExC-3                                                                                                                                                                                                                               | 0.22                 |
| ExC-4                                                                                                                                                                                                                               | 0.02                 |
| Cpd-5                                                                                                                                                                                                                               | $3 \times 10^{-4}$   |
| <u>Layer 4 (2nd Red-Sensitive Emulsion Layer)</u>                                                                                                                                                                                   |                      |
| Silver Iodobromide Emulsion (AgI 4 mol %, high internal AgI type, sphere-corresponding diameter 0.55 $\mu$ m, variation coeff. of sphere-corresponding diameter 20%, normal crystal and twin crystal mixed grains, aspect ratio 1)  | 0.7                  |
| Gelatin                                                                                                                                                                                                                             | 1.26                 |
| ExS-1                                                                                                                                                                                                                               | $1.0 \times 10^{-4}$ |
| ExS-2                                                                                                                                                                                                                               | $3.0 \times 10^{-4}$ |
| ExS-3                                                                                                                                                                                                                               | $1 \times 10^{-5}$   |
| ExC-3                                                                                                                                                                                                                               | 0.33                 |
| ExC-4                                                                                                                                                                                                                               | 0.01                 |
| ExY-16                                                                                                                                                                                                                              | 0.01                 |
| ExC-7                                                                                                                                                                                                                               | 0.04                 |
| ExC-2                                                                                                                                                                                                                               | 0.08                 |
| Solv-1                                                                                                                                                                                                                              | 0.03                 |
| Cpd-5                                                                                                                                                                                                                               | $5 \times 10^{-4}$   |
| <u>Layer 5 (3rd Red-Sensitive Emulsion Layer)</u>                                                                                                                                                                                   |                      |
| Silver Iodobromide Emulsion (AgI 10 mol %, high internal AgI type, sphere-corresponding diameter 0.7 $\mu$ m, variation coeff. of sphere-corresponding diameter 30%, normal crystal and twin crystal mixed grains, aspect ratio 2)  | 0.7                  |

-continued

|                                                                                                                                                                                                                                         |                      |    |
|-----------------------------------------------------------------------------------------------------------------------------------------------------------------------------------------------------------------------------------------|----------------------|----|
| Gelatin                                                                                                                                                                                                                                 | 0.8                  |    |
| ExS-1                                                                                                                                                                                                                                   | $1 \times 10^{-4}$   |    |
| ExS-2                                                                                                                                                                                                                                   | $3 \times 10^{-4}$   |    |
| ExS-3                                                                                                                                                                                                                                   | $1 \times 10^{-5}$   |    |
| ExC-5                                                                                                                                                                                                                                   | 0.05                 |    |
| ExC-6                                                                                                                                                                                                                                   | 0.06                 |    |
| Solv-1                                                                                                                                                                                                                                  | 0.15                 |    |
| Solv-2                                                                                                                                                                                                                                  | 0.08                 |    |
| Cpd-5                                                                                                                                                                                                                                   | $3 \times 10^{-5}$   |    |
| <u>Layer 6 (Interlayer)</u>                                                                                                                                                                                                             |                      |    |
| Gelatin                                                                                                                                                                                                                                 | 1.0                  | 10 |
| Cpd-5                                                                                                                                                                                                                                   | $4 \times 10^{-4}$   |    |
| Cpd-1                                                                                                                                                                                                                                   | 0.10                 |    |
| Cpd-4                                                                                                                                                                                                                                   | 1.23                 |    |
| Solv-1                                                                                                                                                                                                                                  | 0.05                 |    |
| Cpd-3                                                                                                                                                                                                                                   | 0.25                 | 15 |
| <u>Layer 7 (1st Green-Sensitive Emulsion Layer)</u>                                                                                                                                                                                     |                      |    |
| Silver Iodobromide Emulsion (AgI 2 mol %, high internal AgI type, sphere-corresponding diameter 0.3 $\mu\text{m}$ , variation coeff. of sphere-corresponding diameter 28%, normal crystal-twin crystal mixed grains, aspect ratio 2.5)  | 0.30                 |    |
| Gelatin                                                                                                                                                                                                                                 | 0.4                  |    |
| ExS-4                                                                                                                                                                                                                                   | $5 \times 10^{-4}$   |    |
| ExS-6                                                                                                                                                                                                                                   | $0.3 \times 10^{-4}$ |    |
| ExS-5                                                                                                                                                                                                                                   | $2 \times 10^{-4}$   | 20 |
| ExM-9                                                                                                                                                                                                                                   | 0.2                  |    |
| ExY-14                                                                                                                                                                                                                                  | 0.03                 |    |
| ExY-8                                                                                                                                                                                                                                   | 0.03                 |    |
| Solv-1                                                                                                                                                                                                                                  | 0.2                  |    |
| Cpd-5                                                                                                                                                                                                                                   | $2 \times 10^{-4}$   |    |
| <u>Layer 8 (2nd Green-Sensitive Emulsion Layer)</u>                                                                                                                                                                                     |                      | 30 |
| Silver Iodobromide Emulsion (AgI 4 mol %, high internal AgI type, sphere-corresponding diameter 0.55 $\mu\text{m}$ , variation coeff. of sphere-corresponding diameter 20%, normal crystal-twin crystal mixed grains, aspect ratio 4)   | 0.6                  |    |
| Gelatin                                                                                                                                                                                                                                 | 0.8                  |    |
| ExS-4                                                                                                                                                                                                                                   | $5 \times 10^{-4}$   |    |
| ExS-5                                                                                                                                                                                                                                   | $2 \times 10^{-4}$   |    |
| ExS-6                                                                                                                                                                                                                                   | $0.3 \times 10^{-4}$ |    |
| ExM-9                                                                                                                                                                                                                                   | 0.25                 |    |
| ExM-8                                                                                                                                                                                                                                   | 0.03                 |    |
| ExM-10                                                                                                                                                                                                                                  | 0.015                | 40 |
| ExY-14                                                                                                                                                                                                                                  | 0.04                 |    |
| Solv-1                                                                                                                                                                                                                                  | 0.2                  |    |
| Cpd-5                                                                                                                                                                                                                                   | $3 \times 10^{-4}$   |    |
| <u>Layer 9 (3rd Green-Sensitive Emulsion Layer)</u>                                                                                                                                                                                     |                      |    |
| Silver Iodobromide Emulsion (AgI 10 mol %, high internal AgI type, sphere-corresponding diameter 0.7 $\mu\text{m}$ , variation coeff. of sphere-corresponding diameter 30%, normal crystal-twin crystal mixed grains, aspect ratio 2.0) | 0.85                 | 45 |
| Gelatin                                                                                                                                                                                                                                 | 1.0                  |    |
| ExS-4                                                                                                                                                                                                                                   | $2.0 \times 10^{-4}$ |    |
| ExS-5                                                                                                                                                                                                                                   | $2.0 \times 10^{-4}$ |    |
| ExS-6                                                                                                                                                                                                                                   | $0.2 \times 10^{-4}$ |    |

-continued

|                                                                                                                                                                                                                                         |                      |     |
|-----------------------------------------------------------------------------------------------------------------------------------------------------------------------------------------------------------------------------------------|----------------------|-----|
| ExS-7                                                                                                                                                                                                                                   | $3.0 \times 10^{-4}$ |     |
| ExM-12                                                                                                                                                                                                                                  | 0.06                 |     |
| ExM-13                                                                                                                                                                                                                                  | 0.02                 |     |
| ExM-8                                                                                                                                                                                                                                   | 0.02                 |     |
| Solv-1                                                                                                                                                                                                                                  | 0.20                 |     |
| Solv-2                                                                                                                                                                                                                                  | 0.05                 |     |
| Cpd-5                                                                                                                                                                                                                                   | $4 \times 10^{-4}$   |     |
| <u>Layer 10 (Yellow Filter Layer)</u>                                                                                                                                                                                                   |                      |     |
| Gelatin                                                                                                                                                                                                                                 | 0.9                  |     |
| Yellow Colloidal Silver                                                                                                                                                                                                                 | 0.05                 |     |
| Cpd-1                                                                                                                                                                                                                                   | 0.2                  |     |
| Solv-1                                                                                                                                                                                                                                  | 0.15                 |     |
| Cpd-5                                                                                                                                                                                                                                   | $4 \times 10^{-4}$   |     |
| <u>Layer 11 (1st Blue-Sensitive Emulsion Layer)</u>                                                                                                                                                                                     |                      | 0.4 |
| Silver Iodobromide Emulsion (AgI 4 mol %, high internal AgI type, sphere-corresponding diameter 0.5 $\mu\text{m}$ , variation coeff. of sphere-corresponding diameter 15%, octahedral grains)                                           |                      |     |
| Gelatin                                                                                                                                                                                                                                 | 1.0                  |     |
| ExS-8                                                                                                                                                                                                                                   | $2 \times 10^{-4}$   |     |
| ExY-16                                                                                                                                                                                                                                  | 0.9                  |     |
| ExY-14                                                                                                                                                                                                                                  | 0.09                 |     |
| Solv-1                                                                                                                                                                                                                                  | 0.3                  |     |
| Cpd-5                                                                                                                                                                                                                                   | $4 \times 10^{-4}$   |     |
| <u>Layer 12 (2nd Blue-Sensitive Emulsion Layer)</u>                                                                                                                                                                                     |                      |     |
| Silver Iodobromide Emulsion (AgI 10 mol %, high internal AgI type, sphere-corresponding diameter 1.3 $\mu\text{m}$ , variation coeff. of sphere-corresponding diameter 25%, normal crystal-twin crystal mixed grains, aspect ratio 4.5) |                      | 0.5 |
| Gelatin                                                                                                                                                                                                                                 | 0.6                  |     |
| ExS-8                                                                                                                                                                                                                                   | $1 \times 10^{-4}$   |     |
| ExY-16                                                                                                                                                                                                                                  | 0.12                 |     |
| Solv-1                                                                                                                                                                                                                                  | 0.04                 |     |
| Cpd-5                                                                                                                                                                                                                                   | $2 \times 10^{-4}$   |     |
| <u>Layer 13 (1st Protective Layer)</u>                                                                                                                                                                                                  |                      |     |
| Fine Grain Silver Iodobromide (mean grain size 0.07 $\mu\text{m}$ , AgI 1 mol %)                                                                                                                                                        |                      | 0.2 |
| Gelatin                                                                                                                                                                                                                                 | 0.8                  |     |
| UV-3                                                                                                                                                                                                                                    | 0.1                  |     |
| UV-4                                                                                                                                                                                                                                    | 0.1                  |     |
| UV-5                                                                                                                                                                                                                                    | 0.2                  |     |
| Solv-3                                                                                                                                                                                                                                  | 0.04                 |     |
| Cpd-5                                                                                                                                                                                                                                   | $3 \times 10^{-4}$   |     |
| <u>Layer 14 (2nd Protective Layer)</u>                                                                                                                                                                                                  |                      |     |
| Gelatin                                                                                                                                                                                                                                 | 0.9                  |     |
| Polymethyl Methacrylate Particles (diameter 1.5 $\mu\text{m}$ )                                                                                                                                                                         |                      | 0.2 |
| Cpd-5                                                                                                                                                                                                                                   | $4 \times 10^{-4}$   |     |
| H-1                                                                                                                                                                                                                                     | 0.4                  |     |

Each layer further contained a surface active agent as a coating aid in addition to the above components.

The chemical structural formulae or chemical names of the compounds used to prepare the photographic material are shown below.



$x/y = 7/3$  (by weight ratio)



5,338,648

31



32

-continued

UV-1



UV-2



UV-3

Solv-1: Tricresyl Phosphate

Solv-2: Dibutyl Phthalate

Solv-3: Bis(2-ethylhexyl) Phthalate

ExM-8:



ExF-1:



ExC-2:



ExC-3:

-continued



ExY-14:



ExC-4:



ExY-15:



ExC-5:



ExC-6:

-continued



ExC-7:



ExM-9:



ExM-10:



ExM-12:



37

5,338,648

38

-continued

ExM-13:



ExM-16:



Cpd-1:



Cpd-2:



ExS-1:



ExS-2:



ExS-3:

-continued



ExS-4:



ExS-5:



ExS-6:



ExC-7:



ExC-8:



H-1:



Cpd-3:



Cpd-4:



-continued



In addition, the dry thickness of the coated layers of sample 101 excluding the support and the subbing layer on the support was 17.6  $\mu\text{m}$  and the swelling speed ( $T_2$ ) was 8 seconds.

The sample thus prepared was slit to 35 mm in width. After applying an imagewise exposure, the sample was continuously processed by the following processing steps using an automatic processor until the accumulated replenisher amount for the fix solution reached three times the tank volume (i.e., running processing).

| Processing Step   |                 |                       |                              |             |  |
|-------------------|-----------------|-----------------------|------------------------------|-------------|--|
| Step              | Processing Time | Proc-<br>essing Temp. | Replenish-<br>ing Amount     | Tank Volume |  |
| Color Development | 3 min. 15 sec.  | 38° C.                | 15 ml                        | 20 liters   |  |
| Bleach            | 4 min. 30 sec.  | 38° C.                | 10 ml                        | 40 liters   |  |
| Wash              | 2 min. 10 sec.  | 35° C.                | 10 ml                        | 20 liters   |  |
| Fix               | 4 min. 20 sec.  | 38° C.                | (1) 30 ml<br>or<br>(2) 15 ml | 30 liters   |  |
| Wash (1)          | 65 sec.         | 35° C.                | (*)                          | 10 liters   |  |
| Wash (2)          | 1 min.          | 35° C.                | 20 ml                        | 10 liters   |  |
| Stabilizing       | 65 sec.         | 38° C.                | 10 ml                        | 10 liters   |  |
| Drying            | 4 min. 20 sec.  | 55° C.                |                              |             |  |

(\*): Counter-current system from (2) to (1).

The replenishing amount was per 1 meter in length (35 mm in width) of the photographic material processed.

The composition of each processing solution is shown below.

|                                                                   | Tank    | Replenisher |
|-------------------------------------------------------------------|---------|-------------|
| <u>Color Developer</u>                                            |         |             |
| Diethylenetriaminepentaacetic Acid                                | 1.0 g   | 1.1 g       |
| 1-Hydroxyethylidene-1,1-di-phosphonic Acid                        | 3.0 g   | 3.2 g       |
| Sodium Sulfite                                                    | 4.0 g   | 4.9 g       |
| Potassium Carbonate                                               | 30.0 g  | 30.0 g      |
| Potassium Bromide                                                 | 1.4 g   | —           |
| Potassium Iodide                                                  | 1.5 mg  | —           |
| Hydroxylamine Sulfate                                             | 2.4 g   | 3.6 g       |
| 4-(N-Ethyl-N-β-hydroxyethyl-amino)-2-methylaniline Sulfate        | 4.5 g   | 7.2 g       |
| Water to make                                                     | 1 liter | 1 liter     |
| pH                                                                | 10.05   | 10.10       |
| <u>Bleach Solution</u>                                            |         |             |
| 1,3-Propylenediaminetetra-acetic Acid Ferric Ammonium Monohydrate | 144.0 g | 206.0 g     |
| Ammonium Bromide                                                  | 84.0 g  | 120.0 g     |
| Ammonium Nitrate                                                  | 30.0 g  | 41.7 g      |
| Acetic Acid (98 wt %)                                             | 28.0 g  | 40.0 g      |
| Hydroxyacetic Acid                                                | 63.0 g  | 90.0 g      |
| Water to make                                                     | 1 liter | 1 liter     |
| pH (adjusted by aqueous ammonia (27 wt %))                        | 3.0     | 2.8         |

-continued

|                                                                                                         | Tank     | Replenisher |
|---------------------------------------------------------------------------------------------------------|----------|-------------|
| <u>Fix Solution</u>                                                                                     |          |             |
| Ethylenediaminetetraacetic Acid Disodium Salt                                                           | 0.5 g    | 1.0 g       |
| Sodium Sulfite                                                                                          | 7.0 g    | 12.0 g      |
| Sodium Bisulfite                                                                                        | 5.0 g    | 9.5 g       |
| Fixing Agent: Aqueous solution of Ammonium Thiosulfate (70 wt %) or Fixing Agent shown in Table 1 below | 170.0 ml | 240.0 ml    |
| Water to make                                                                                           | 0.8 mol  | 1.1 mol     |
| pH                                                                                                      | 1 liter  | 1 liter     |
| Wash Water Tank = Replenisher                                                                           | 6.7      | 6.7         |

25 City water was passed through a mixed bed column packed with a H-type strong acidic cation exchange resin (Amberlite IR-120B, trade name, made by Rohm & Haas Company) and a OH-type anion exchange resin (Amberlite IR-400, trade name) to reduce the calcium 30 ion and magnesium ion concentrations below 3 mg/liter. Then, 20 mg/liter of dichloro sodium isocyanurate and 0.15 g/liter of sodium sulfate were added thereto. The pH of the solution was in the range of from 6.5 to 7.5.

| Stabilization solution                                                    | Tank    | Replenisher |
|---------------------------------------------------------------------------|---------|-------------|
| Formalin (37 wt %)                                                        | 2.0 ml  | 3.0 ml      |
| Polyoxyethylene-p-mononyl-phenyl Ether (average polymerization degree 10) | 0.3 g   | 0.45 g      |
| Ethylenediaminetetraacetic Acid Disodium Salt                             | 0.05    | 0.08        |
| Water to make                                                             | 1 liter | 1 liter     |
| pH                                                                        | 5.0-8.0 | 5.0-8.0     |

After the completion of running processing, the same sample type as used for the running processing was processed as described above, except that the fixing time was shortened to 2 minutes or 3 minutes.

50 The residual salver amount at the unexposed portions of the sample thus processed was measured using a fluroescent X ray analyzer.

Also, the extent of precipitations in the fix bath and wash bath (1) were visually evaluated.

55 The results obtained are shown in Table 1.  
From the results shown in Table 1, it is clearly seen  
that when the compound of formula (I) of this invention  
was used, the liquid stability was excellent without  
precipitation in the running processing. Furthermore,  
60 desilvering was complete at a fixing time of 3 minutes,  
which clearly shows that the fixing ability of the com-  
pound of formula (I) of this invention is superior to that  
of a thiosulfate. Also, the effect of this invention was  
particularly remarkable when the replenishing amount  
65 was reduced.

TABLE 1

| Fixing Agent | Replenishing Amount for Fix Bath | Residual Silver Amount ( $\mu\text{g}/\text{cm}^2$ ) |              | Presence of Precipitation in Fix Bath | Presence of Precipitation in Wash Bath | Comparison |
|--------------|----------------------------------|------------------------------------------------------|--------------|---------------------------------------|----------------------------------------|------------|
|              |                                  | Fixed 2 min.                                         | Fixed 3 min. |                                       |                                        |            |
| Ammonium     | (1)                              | 25                                                   | 4.0          | Δ                                     | Δ                                      |            |
| Thiosulfate  | (2)                              | 35                                                   | 8.5          | X                                     | X                                      |            |
| Compound-1   | (1)                              | 11                                                   | 0.8          | ○                                     | ○                                      | Invention  |
|              | (2)                              | 15                                                   | 1.1          | ○○                                    | ○○                                     |            |
| Compound-4   | (1)                              | 13                                                   | 0.9          | ○○                                    | ○○                                     | Invention  |
|              | (2)                              | 15                                                   | 1.1          | ○○                                    | ○○                                     |            |
| Compound-18  | (1)                              | 10                                                   | 0.7          | ○○                                    | ○○                                     | Invention  |
|              | (2)                              | 16                                                   | 1.0          | ○○                                    | ○○                                     |            |
| Compound-19  | (1)                              | 11                                                   | 0.8          | ○○                                    | ○○                                     | Invention  |
|              | (2)                              | 18                                                   | 1.1          | ○○                                    | ○○                                     |            |

Evaluation of the presence of precipitations:

○: No precipitation by visual observation  
 Δ: Small amount of precipitation  
 X: Large amount of precipitation

### EXAMPLE 2

The procedure of Example 1 was repeated, except for using Compound-2, 3, 9, 12, 13, 14, 20, 23, 25, 26, or 32 in place of Compound-1 in Example 1. In each case, good results were obtained as in Example 1; namely, the fixing ability was high and the precipitates were not formed in the running processing. Also, the effects of the invention were pronounced when the replenishing amount was reduced.

### EXAMPLE 3

A multilayer color photographic paper having the layer structure shown below was prepared on a paper support, both surfaces of which were coated with polyethylene. The coating compositions were prepared as follows.

#### Preparation of Coating Composition for Layer 1

In 27.2 ml of ethyl acetate and 8.2 g of a solvent (solv-1) were dissolved 19.1 g of a yellow coupler (exY), 4.4 g of a color image stabilizer (cpd-1), and 0.7 g of a color image stabilizer (cpd-7), and the solution obtained was dispersed by emulsification in 185 ml of an aqueous 10 wt % gelatin solution containing 8 ml of an aqueous solution of 10 wt % sodium dodecylbenzenesulfonate.

On the other hand, to a silver chlorobromide emulsion (cubic, a 3:7 mixture (by mol ratio of silver) of large size emulsion having a mean grain size of 0.88  $\mu\text{m}$  and a

20  
 25  
 30  
 35  
 40  
 45  
 50  
 55  
 60  
 65  
 70  
 75  
 80  
 85  
 90  
 95  
 100  
 105  
 110  
 115  
 120  
 125  
 130  
 135  
 140  
 145  
 150  
 155  
 160  
 165  
 170  
 175  
 180  
 185  
 190  
 195  
 200  
 205  
 210  
 215  
 220  
 225  
 230  
 235  
 240  
 245  
 250  
 255  
 260  
 265  
 270  
 275  
 280  
 285  
 290  
 295  
 300  
 305  
 310  
 315  
 320  
 325  
 330  
 335  
 340  
 345  
 350  
 355  
 360  
 365  
 370  
 375  
 380  
 385  
 390  
 395  
 400  
 405  
 410  
 415  
 420  
 425  
 430  
 435  
 440  
 445  
 450  
 455  
 460  
 465  
 470  
 475  
 480  
 485  
 490  
 495  
 500  
 505  
 510  
 515  
 520  
 525  
 530  
 535  
 540  
 545  
 550  
 555  
 560  
 565  
 570  
 575  
 580  
 585  
 590  
 595  
 600  
 605  
 610  
 615  
 620  
 625  
 630  
 635  
 640  
 645  
 650  
 655  
 660  
 665  
 670  
 675  
 680  
 685  
 690  
 695  
 700  
 705  
 710  
 715  
 720  
 725  
 730  
 735  
 740  
 745  
 750  
 755  
 760  
 765  
 770  
 775  
 780  
 785  
 790  
 795  
 800  
 805  
 810  
 815  
 820  
 825  
 830  
 835  
 840  
 845  
 850  
 855  
 860  
 865  
 870  
 875  
 880  
 885  
 890  
 895  
 900  
 905  
 910  
 915  
 920  
 925  
 930  
 935  
 940  
 945  
 950  
 955  
 960  
 965  
 970  
 975  
 980  
 985  
 990  
 995  
 1000  
 1005  
 1010  
 1015  
 1020  
 1025  
 1030  
 1035  
 1040  
 1045  
 1050  
 1055  
 1060  
 1065  
 1070  
 1075  
 1080  
 1085  
 1090  
 1095  
 1100  
 1105  
 1110  
 1115  
 1120  
 1125  
 1130  
 1135  
 1140  
 1145  
 1150  
 1155  
 1160  
 1165  
 1170  
 1175  
 1180  
 1185  
 1190  
 1195  
 1200  
 1205  
 1210  
 1215  
 1220  
 1225  
 1230  
 1235  
 1240  
 1245  
 1250  
 1255  
 1260  
 1265  
 1270  
 1275  
 1280  
 1285  
 1290  
 1295  
 1300  
 1305  
 1310  
 1315  
 1320  
 1325  
 1330  
 1335  
 1340  
 1345  
 1350  
 1355  
 1360  
 1365  
 1370  
 1375  
 1380  
 1385  
 1390  
 1395  
 1400  
 1405  
 1410  
 1415  
 1420  
 1425  
 1430  
 1435  
 1440  
 1445  
 1450  
 1455  
 1460  
 1465  
 1470  
 1475  
 1480  
 1485  
 1490  
 1495  
 1500  
 1505  
 1510  
 1515  
 1520  
 1525  
 1530  
 1535  
 1540  
 1545  
 1550  
 1555  
 1560  
 1565  
 1570  
 1575  
 1580  
 1585  
 1590  
 1595  
 1600  
 1605  
 1610  
 1615  
 1620  
 1625  
 1630  
 1635  
 1640  
 1645  
 1650  
 1655  
 1660  
 1665  
 1670  
 1675  
 1680  
 1685  
 1690  
 1695  
 1700  
 1705  
 1710  
 1715  
 1720  
 1725  
 1730  
 1735  
 1740  
 1745  
 1750  
 1755  
 1760  
 1765  
 1770  
 1775  
 1780  
 1785  
 1790  
 1795  
 1800  
 1805  
 1810  
 1815  
 1820  
 1825  
 1830  
 1835  
 1840  
 1845  
 1850  
 1855  
 1860  
 1865  
 1870  
 1875  
 1880  
 1885  
 1890  
 1895  
 1900  
 1905  
 1910  
 1915  
 1920  
 1925  
 1930  
 1935  
 1940  
 1945  
 1950  
 1955  
 1960  
 1965  
 1970  
 1975  
 1980  
 1985  
 1990  
 1995  
 2000  
 2005  
 2010  
 2015  
 2020  
 2025  
 2030  
 2035  
 2040  
 2045  
 2050  
 2055  
 2060  
 2065  
 2070  
 2075  
 2080  
 2085  
 2090  
 2095  
 2100  
 2105  
 2110  
 2115  
 2120  
 2125  
 2130  
 2135  
 2140  
 2145  
 2150  
 2155  
 2160  
 2165  
 2170  
 2175  
 2180  
 2185  
 2190  
 2195  
 2200  
 2205  
 2210  
 2215  
 2220  
 2225  
 2230  
 2235  
 2240  
 2245  
 2250  
 2255  
 2260  
 2265  
 2270  
 2275  
 2280  
 2285  
 2290  
 2295  
 2300  
 2305  
 2310  
 2315  
 2320  
 2325  
 2330  
 2335  
 2340  
 2345  
 2350  
 2355  
 2360  
 2365  
 2370  
 2375  
 2380  
 2385  
 2390  
 2395  
 2400  
 2405  
 2410  
 2415  
 2420  
 2425  
 2430  
 2435  
 2440  
 2445  
 2450  
 2455  
 2460  
 2465  
 2470  
 2475  
 2480  
 2485  
 2490  
 2495  
 2500  
 2505  
 2510  
 2515  
 2520  
 2525  
 2530  
 2535  
 2540  
 2545  
 2550  
 2555  
 2560  
 2565  
 2570  
 2575  
 2580  
 2585  
 2590  
 2595  
 2600  
 2605  
 2610  
 2615  
 2620  
 2625  
 2630  
 2635  
 2640  
 2645  
 2650  
 2655  
 2660  
 2665  
 2670  
 2675  
 2680  
 2685  
 2690  
 2695  
 2700  
 2705  
 2710  
 2715  
 2720  
 2725  
 2730  
 2735  
 2740  
 2745  
 2750  
 2755  
 2760  
 2765  
 2770  
 2775  
 2780  
 2785  
 2790  
 2795  
 2800  
 2805  
 2810  
 2815  
 2820  
 2825  
 2830  
 2835  
 2840  
 2845  
 2850  
 2855  
 2860  
 2865  
 2870  
 2875  
 2880  
 2885  
 2890  
 2895  
 2900  
 2905  
 2910  
 2915  
 2920  
 2925  
 2930  
 2935  
 2940  
 2945  
 2950  
 2955  
 2960  
 2965  
 2970  
 2975  
 2980  
 2985  
 2990  
 2995  
 3000  
 3005  
 3010  
 3015  
 3020  
 3025  
 3030  
 3035  
 3040  
 3045  
 3050  
 3055  
 3060  
 3065  
 3070  
 3075  
 3080  
 3085  
 3090  
 3095  
 3100  
 3105  
 3110  
 3115  
 3120  
 3125  
 3130  
 3135  
 3140  
 3145  
 3150  
 3155  
 3160  
 3165  
 3170  
 3175  
 3180  
 3185  
 3190  
 3195  
 3200  
 3205  
 3210  
 3215  
 3220  
 3225  
 3230  
 3235  
 3240  
 3245  
 3250  
 3255  
 3260  
 3265  
 3270  
 3275  
 3280  
 3285  
 3290  
 3295  
 3300  
 3305  
 3310  
 3315  
 3320  
 3325  
 3330  
 3335  
 3340  
 3345  
 3350  
 3355  
 3360  
 3365  
 3370  
 3375  
 3380  
 3385  
 3390  
 3395  
 3400  
 3405  
 3410  
 3415  
 3420  
 3425  
 3430  
 3435  
 3440  
 3445  
 3450  
 3455  
 3460  
 3465  
 3470  
 3475  
 3480  
 3485  
 3490  
 3495  
 3500  
 3505  
 3510  
 3515  
 3520  
 3525  
 3530  
 3535  
 3540  
 3545  
 3550  
 3555  
 3560  
 3565  
 3570  
 3575  
 3580  
 3585  
 3590  
 3595  
 3600  
 3605  
 3610  
 3615  
 3620  
 3625  
 3630  
 3635  
 3640  
 3645  
 3650  
 3655  
 3660  
 3665  
 3670  
 3675  
 3680  
 3685  
 3690  
 3695  
 3700  
 3705  
 3710  
 3715  
 3720  
 3725  
 3730  
 3735  
 3740  
 3745  
 3750  
 3755  
 3760  
 3765  
 3770  
 3775  
 3780  
 3785  
 3790  
 3795  
 3800  
 3805  
 3810  
 3815  
 3820  
 3825  
 3830  
 3835  
 3840  
 3845  
 3850  
 3855  
 3860  
 3865  
 3870  
 3875  
 3880  
 3885  
 3890  
 3895  
 3900  
 3905  
 3910  
 3915  
 3920  
 3925  
 3930  
 3935  
 3940  
 3945  
 3950  
 3955  
 3960  
 3965  
 3970  
 3975  
 3980  
 3985  
 3990  
 3995  
 4000  
 4005  
 4010  
 4015  
 4020  
 4025  
 4030  
 4035  
 4040  
 4045  
 4050  
 4055  
 4060  
 4065  
 4070  
 4075  
 4080  
 4085  
 4090  
 4095  
 4100  
 4105  
 4110  
 4115  
 4120  
 4125  
 4130  
 4135  
 4140  
 4145  
 4150  
 4155  
 4160  
 4165  
 4170  
 4175  
 4180  
 4185  
 4190  
 4195  
 4200  
 4205  
 4210  
 4215  
 4220  
 4225  
 4230  
 4235  
 4240  
 4245  
 4250  
 4255  
 4260  
 4265  
 4270  
 4275  
 4280  
 4285  
 4290  
 4295  
 4300  
 4305  
 4310  
 4315  
 4320  
 4325  
 4330  
 4335  
 4340  
 4345  
 4350  
 4355  
 4360  
 4365  
 4370  
 4375  
 4380  
 4385  
 4390  
 4395  
 4400  
 4405  
 4410  
 4415  
 4420  
 4425  
 4430  
 4435  
 4440  
 4445  
 4450  
 4455  
 4460  
 4465  
 4470  
 4475  
 4480  
 4485  
 4490  
 4495  
 4500  
 4505  
 4510  
 4515  
 4520  
 4525  
 4530  
 4535  
 4540  
 4545  
 4550  
 4555  
 4560  
 4565  
 4570  
 4575  
 4580  
 4585  
 4590  
 4595  
 4600  
 4605  
 4610  
 4615  
 4620  
 4625  
 4630  
 4635  
 4640  
 4645  
 4650  
 4655  
 4660  
 4665  
 4670  
 4675  
 4680  
 4685  
 4690  
 4695  
 4700  
 4705  
 4710  
 4715  
 4720  
 4725  
 4730  
 4735  
 4740  
 4745  
 4750  
 4755  
 4760  
 4765  
 4770  
 4775  
 4780  
 4785  
 4790  
 4795  
 4800  
 4805  
 4810  
 4815  
 4820  
 4825  
 4830  
 4835  
 4840  
 4845  
 4850  
 4855  
 4860  
 4865  
 4870  
 4875  
 4880  
 4885  
 4890  
 4895  
 4900  
 4905  
 4910  
 4915  
 4920  
 4925  
 4930  
 4935  
 4940  
 4945  
 4950  
 4955  
 4960  
 4965  
 4970  
 4975  
 4980  
 4985  
 4990  
 4995  
 5000  
 5005  
 5010  
 5015  
 5020  
 5025  
 5030  
 5035  
 5040  
 5045  
 5050  
 5055  
 5060  
 5065  
 5070  
 5075  
 5080  
 5085  
 5090  
 5095  
 5100  
 5105  
 5110  
 5115  
 5120  
 5125  
 5130  
 5135  
 5140  
 5145  
 5150  
 5155  
 5160  
 5165  
 5170  
 5175  
 5180  
 5185  
 5190  
 5195  
 5200  
 5205  
 5210  
 5215  
 5220  
 5225  
 5230  
 5235  
 5240  
 5245  
 5250  
 5255  
 5260  
 5265  
 5270  
 5275  
 5280  
 5285  
 5290  
 5295  
 5300  
 5305  
 5310  
 5315  
 5320  
 5325  
 5330  
 5335  
 5340  
 5345  
 5350  
 5355  
 5360  
 5365  
 5370  
 5375  
 5380  
 5385  
 5390  
 5395  
 5400  
 5405  
 5410  
 5415  
 5420  
 5425  
 5430  
 5435  
 5440  
 5445  
 5450  
 5455  
 5460  
 5465  
 5470  
 5475  
 5480  
 5485  
 5490  
 5495  
 5500  
 5505  
 5510  
 5515  
 5520  
 5525  
 5530  
 5535  
 5540  
 5545  
 5550  
 5555  
 5560  
 5565  
 5570  
 5575  
 5580  
 5585  
 5590  
 5595  
 5600  
 5605  
 5610  
 5615  
 5620  
 5625  
 5630  
 5635  
 5640  
 5645  
 5650  
 5655  
 5660  
 5665  
 5670  
 5675  
 5680  
 5685  
 5690  
 5695  
 5700  
 5705  
 5710  
 5715  
 5720  
 5725  
 5730  
 5735  
 5740  
 5745  
 5750  
 5755  
 5760  
 5765  
 5770  
 5775  
 5780  
 5785  
 5790  
 5795  
 5800  
 5805  
 5810  
 5815  
 5820  
 5825  
 5830  
 5835  
 5840  
 5845  
 5850  
 5855  
 5860  
 5865  
 5870  
 5875  
 5880  
 5885  
 5890  
 5895  
 5900  
 5905  
 5910  
 5915  
 5920  
 5925  
 5930  
 5935  
 5940  
 5945  
 5950  
 5955  
 5960  
 5965  
 5970  
 5975  
 5980  
 5985  
 5990



5 (7.0  $\times 10^{-5}$  mol added to the large size emulsion and 10 mol added to the small size emulsion per mol of silver halide).

totetrazole in amounts of 8.5  $\times 10^{-5}$  mol, 7.7  $\times 10^{-4}$  mol, and 2.5  $\times 10^{-4}$  mol, respectively per mol of silver halide.

Furthermore, to the blue-sensitive emulsion layer and the green-sensitive emulsion layer was added 4-hydroxy-6-methyl-1,3,3a,7-tetraazaindene in amounts of 1  $\times 10^{-4}$  mol and 2  $\times 10^{-4}$  mol, respectively, per mol of silver halide.

Also, the following dyes were added to each emulsion layer for irradiation protection.



and



1.0  $\times 10^{-5}$  mol added to the small size emulsion per mol of silver halide).

For the red-sensitive emulsion layer:



(0.9  $\times 10^{-4}$  mol added to the large size emulsion and 1.1  $\times 10^{-4}$  mol added to the small size emulsion per mol of silver halide).

Also, to the red-sensitive emulsion layer was added 50 the following compound in an amount of 2.6  $\times 10^{-3}$  mol per mol of silver halide.

#### Layer Structure

The composition of each layer is shown below. The coating amounts are given in units of (g/m<sup>2</sup>), and the coating amounts for the silver halide emulsion are given in terms of silver.

#### Support

Polyethylene-coated paper ([the polyethylene coating at the emulsion layer side contained a white pigment (TiO<sub>2</sub>) and a bluish dye (ultramarine blue)].

#### Layer 1 (Blue-Sensitive Layer)

|                                               |      |
|-----------------------------------------------|------|
| Above described Silver Chlorobromide Emulsion | 0.30 |
| Gelatin                                       | 1.86 |
| Yellow Coupler (exY)                          | 0.82 |
| Color Image Stabilizer (cpd-1)                | 0.19 |
| Solvent (Solv-1)                              | 0.35 |
| Color Image Stabilizer (cpd-7)                | 0.06 |



Also, to the blue-sensitive emulsion layer, the green-sensitive emulsion layer, and the red-sensitive emulsion layer was added 1-(5-methylureidophenyl)-5-mercaptop-

#### Layer 2 (Color Mixing Inhibition Layer)

|         |      |
|---------|------|
| Gelatin | 0.99 |
|---------|------|

-continued

|                                                                                                                                                                                                                                                                                                                                                                             |      |
|-----------------------------------------------------------------------------------------------------------------------------------------------------------------------------------------------------------------------------------------------------------------------------------------------------------------------------------------------------------------------------|------|
| Color Mixing Inhibitor (cpd-5)                                                                                                                                                                                                                                                                                                                                              | 0.08 |
| Solvent (Solv-1)                                                                                                                                                                                                                                                                                                                                                            | 0.16 |
| Solvent (Solv-4)                                                                                                                                                                                                                                                                                                                                                            | 0.08 |
| <u>Layer 3 (Green-Sensitive Layer)</u>                                                                                                                                                                                                                                                                                                                                      |      |
| Silver Chlorobromide Emulsion (cubic, a:1:3 mixture (by mol ratio of silver) of large size emulsion having a mean grain size of 0.55 $\mu\text{m}$ and small size emulsion having a mean grain size of 0.39 $\mu\text{m}$ , variation coeff. of grain size distribution 0.10 and 0.08, respectively, each emulsion had locally 0.8 mol % AgBr at the surface of the grains) | 0.12 |
| Gelatin                                                                                                                                                                                                                                                                                                                                                                     | 1.24 |
| Magenta Coupler (exM)                                                                                                                                                                                                                                                                                                                                                       | 0.20 |
| Color Image Stabilizer (cpd-2)                                                                                                                                                                                                                                                                                                                                              | 0.03 |
| Color Image Stabilizer (cpd-3)                                                                                                                                                                                                                                                                                                                                              | 0.15 |
| Color Image Stabilizer (cpd-4)                                                                                                                                                                                                                                                                                                                                              | 0.02 |
| Color Image Stabilizer (cpd-9)                                                                                                                                                                                                                                                                                                                                              | 0.02 |
| Solvent (solv-2)                                                                                                                                                                                                                                                                                                                                                            | 0.40 |
| <u>Layer 4 (Ultraviolet Absorption Layer)</u>                                                                                                                                                                                                                                                                                                                               |      |
| Gelatin                                                                                                                                                                                                                                                                                                                                                                     | 1.58 |
| Ultraviolet Absorbent (uv-1)                                                                                                                                                                                                                                                                                                                                                | 0.47 |
| Color Mixing Inhibitor (cpd-5)                                                                                                                                                                                                                                                                                                                                              | 0.05 |
| Solvent (solv-5)                                                                                                                                                                                                                                                                                                                                                            | 0.24 |
| <u>Layer 5 (Red-Sensitive Layer)</u>                                                                                                                                                                                                                                                                                                                                        |      |
| Silver Chlorobromide Emulsion (cubic,                                                                                                                                                                                                                                                                                                                                       | 0.23 |

-continued

|                                                                                                                                                                                                                                                                                                                                   |      |
|-----------------------------------------------------------------------------------------------------------------------------------------------------------------------------------------------------------------------------------------------------------------------------------------------------------------------------------|------|
| a 1:4 mixture (by mol ratio of silver) of large size emulsion having a mean grain size of 0.58 $\mu\text{m}$ and small size emulsion having a mean grain size of 0.45 $\mu\text{m}$ , variation coeff. of grain size distribution 0.09 and 0.11, respectively, each emulsion had locally 0.6 mol % AgBr at the surface of grains) |      |
| Gelatin                                                                                                                                                                                                                                                                                                                           | 1.34 |
| Cyan Coupler (exC)                                                                                                                                                                                                                                                                                                                | 0.32 |
| Color Image Stabilizer (cpd 6)                                                                                                                                                                                                                                                                                                    | 0.17 |
| Color Image Stabilizer (cpd-7)                                                                                                                                                                                                                                                                                                    | 0.40 |
| Color Image Stabilizer (cpd-8)                                                                                                                                                                                                                                                                                                    | 0.04 |
| Solvent (solv-6)                                                                                                                                                                                                                                                                                                                  | 0.15 |
| <u>Layer 6 (Ultraviolet Absorption Layer)</u>                                                                                                                                                                                                                                                                                     |      |
| Gelatin                                                                                                                                                                                                                                                                                                                           | 0.53 |
| Ultraviolet Absorbent (uv-1)                                                                                                                                                                                                                                                                                                      | 0.16 |
| Color Mixing Inhibitor (cpd-5)                                                                                                                                                                                                                                                                                                    | 0.02 |
| Solvent (solv-5)                                                                                                                                                                                                                                                                                                                  | 0.08 |
| <u>Layer 7 (Protective Layer)</u>                                                                                                                                                                                                                                                                                                 |      |
| Gelatin                                                                                                                                                                                                                                                                                                                           | 1.33 |
| Acryl-Modified copolymer of Polyvinyl                                                                                                                                                                                                                                                                                             | 0.17 |
| Alcohol (modified degree 17%)                                                                                                                                                                                                                                                                                                     |      |
| Fluid Paraffin                                                                                                                                                                                                                                                                                                                    | 0.03 |

The compounds used for preparing the color photographic paper are shown below.

## (exY) Yellow Coupler:

A 1/1 mixture (by mol ratio) of



## (exM) Magenta Coupler:

A 1/1 mixture (by mol ratio) of



and

-continued



(exC) Cyan Coupler:  
A 2:4:4 mixture (by weight ratio) of



and



(cpd-1) Color Image Stabilizer:



(cpd-2) Color Image Stabilizer:



(cpd-3) Color Image Stabilizer:



(cpd-4) Color Image Stabilizer:



(cpd-5) Color Mixing Inhibitor:

-continued



(cpd-6) Color Image Stabilizer:  
A 2:4:4 mixture (by weight ratio) of



(cpd-7) Color Image Stabilizer:



Average molecular weight 60,000

(cpd-8) Color Image Stabilizer:



(cpd-9) Color Image Stabilizer:



(uv-1) Ultraviolet Absorbent:

A 4:2:4 mixture (by weight ratio) of



-continued



**(solv-1) Solvent:**



**(solv-2) Solvent:**

(Solv-Z) Solvent:  
A 2:1 mixture (by volume) of



**(solv-4) Solvent:**



**(solv-5) Solvent:**

$$\text{COOC}_8\text{H}_{17}$$

1  
(CH<sub>2</sub>)<sub>6</sub>

$\text{CH}_2\text{CH}_2$

4.4.2.6.1



After imagewise exposing the aforesaid color photographic paper, continuous processing (running test) was conducted using a color photographic paper processor and the following processing steps until the replenishing amount for the blix solution reached twice the volume of the blix tank.

-continued

| Processing Step   | Temperature<br>(°C.) | Time<br>(sec.) | Replenish-<br>ing amount | Tank<br>volume<br>(liter) |
|-------------------|----------------------|----------------|--------------------------|---------------------------|
| Color Development | 35                   | 45             | 109 ml                   | 17                        |

| -Continued      |                   |             |                              |                     |
|-----------------|-------------------|-------------|------------------------------|---------------------|
| Processing Step | Temperature (°C.) | Time (sec.) | Replenishing amount          | Tank volume (liter) |
| Blix            | 35                | 45          | (1) 61 ml<br>or<br>(2) 30 ml | 17                  |
| Rinse (1)       | 35                | 30          | —                            | 10                  |
| Rinse (2)       | 35                | 30          | —                            | 10                  |
| Rinse (3)       | 35                | 30          | 300 ml                       | 10                  |

-continued

| Processing Step | Temperature (°C.) | Time (sec.) | Replenishing amount | Tank volume (liter) |
|-----------------|-------------------|-------------|---------------------|---------------------|
| Drying          | 80                | 60          |                     |                     |

## Note

- (1): The replenishing amount was per square meter of the color photographic paper processed.  
 (2): To the blix solution were replenished the replenisher for the blix solution and the rinse (1) solution (121 ml).  
 (3): Three-tank counter-current system of rinse (3) to rinse (1) was used.

The composition of each processing solution was as follows.

| Color Developer | Tank Solution | Replenisher |
|-----------------|---------------|-------------|
|-----------------|---------------|-------------|

| Fixing Agent | Replenishing Amount for Blix Bath | Presence of Precipitation in Blix Bath | Presence of Precipitation in Rinse (1) Bath | Comparison |
|--------------|-----------------------------------|----------------------------------------|---------------------------------------------|------------|
| Ammonium     | (1)                               | Δ                                      | X                                           |            |
| Thiosulfate  | (2)                               | X                                      | XX                                          |            |
| Compound-1   | (1)                               | ○                                      | ○                                           | Invention  |
|              | (2)                               | ○                                      | ○                                           |            |
| Compound-4   | (1)                               | ○                                      | ○                                           | "          |
|              | (2)                               | ○                                      | ○                                           | "          |
| Compound-18  | (1)                               | ○                                      | ○                                           | "          |
|              | (2)                               | ○                                      | ○                                           | "          |
| Compound-19  | (1)                               | ○                                      | ○                                           | "          |
|              | (2)                               | ○                                      | ○                                           | "          |
| Compound-25  | (1)                               | ○                                      | ○                                           | "          |
|              | (2)                               | ○                                      | ○                                           | "          |

## Evaluation of the presence of precipitations:

○: No precipitation by visual observation

Δ: Small amount of precipitation

X: Large amount of precipitation

XX: Very large amount of precipitation

|                                                                                                         | 800 ml        | 800 ml          |
|---------------------------------------------------------------------------------------------------------|---------------|-----------------|
| Water                                                                                                   | 800 ml        | 800 ml          |
| Ethylenediamine-N,N,N,N-tetramethylenephosphonic Acid                                                   | 3.0 g         | 3.0 g           |
| Triethanolamine                                                                                         | 5.0 g         | 5.0 g           |
| Potassium Chloride                                                                                      | 3.1 g         | —               |
| Potassium Bromide                                                                                       | 0.015 g       | —               |
| Potassium Carbonate                                                                                     | 25 g          | 25 g            |
| Hydrazinodiacetic Acid                                                                                  | 5.0 g         | 7.0 g           |
| N-Ethyl-N-(β-methanesulfonamidoethyl)-3-methyl-4-aminoaniline Sulfate                                   | 5.0 g         | 9.5 g           |
| Fluorescent Whitening Agent (Whitex-4, trade name, made by Sumitomo Chemical Company Ltd.)              | 1.0 g         | 2.5 g           |
| Water to make                                                                                           | 1 liter       | 1 liter         |
| pH (with the addition of KOH)                                                                           | 10.05         | 10.60           |
|                                                                                                         | Tank Solution | (1) Replenisher |
|                                                                                                         |               | (2) Replenisher |
| <u>Blix Solution</u>                                                                                    |               |                 |
| Water                                                                                                   | 600 ml        | 150 ml          |
| Ammonium Thiosulfate (70 wt %) or the compound of this Invention (formula (I)) as indicated in Table 2. | 100 ml        | 245 ml          |
|                                                                                                         | 0.4 mol       | 1.0 mol         |
| Ammonium Sulfite                                                                                        | 45 g          | 105 g           |
| Ethylenediamine-tetraacetic Acid                                                                        | 55 g          | 135 g           |
| Iron(III) Ammonium Salt                                                                                 | 3.0 g         | 8.0 g           |
| Ethylenediamine-tetraacetic Acid                                                                        | 3.0 g         | 8.0 g           |
| Ammonium Bromide                                                                                        | 30 g          | 75 g            |
| Nitric Acid (67 wt %)                                                                                   | 27 g          | 68 g            |
| Water to make                                                                                           | 1 liter       | 1 liter         |
| pH                                                                                                      | 5.80          | 5.60            |
|                                                                                                         |               | 5.40            |

-continued

## Rinse Solution (Tank solution = Replenisher)

- 5 Ion-exchanged water (each of calcium ion and magnesium ion concentrations being less than 3 ppm). After finishing the running process, the presence of precipitation in the rinse (1) bath was visually evaluated.
- 10 The results obtained are shown in Table 2. From the results shown in Table 2, it is clearly seen that when the compound of formula (I) of this invention is used in place of the thiosulfate, the liquid stability is excellent without precipitation in the running processing. Also, the effect of this invention is pronounced when the amount of the replenisher is reduced.

TABLE 2

| Fixing Agent | Replenishing Amount for Blix Bath | Presence of Precipitation in Blix Bath | Presence of Precipitation in Rinse (1) Bath | Comparison |
|--------------|-----------------------------------|----------------------------------------|---------------------------------------------|------------|
| Ammonium     | (1)                               | Δ                                      | X                                           |            |
| Thiosulfate  | (2)                               | X                                      | XX                                          |            |
| Compound-1   | (1)                               | ○                                      | ○                                           | Invention  |
|              | (2)                               | ○                                      | ○                                           |            |
| Compound-4   | (1)                               | ○                                      | ○                                           | "          |
|              | (2)                               | ○                                      | ○                                           | "          |
| Compound-18  | (1)                               | ○                                      | ○                                           | "          |
|              | (2)                               | ○                                      | ○                                           | "          |
| Compound-19  | (1)                               | ○                                      | ○                                           | "          |
|              | (2)                               | ○                                      | ○                                           | "          |
| Compound-25  | (1)                               | ○                                      | ○                                           | "          |
|              | (2)                               | ○                                      | ○                                           | "          |

## EXAMPLE 4

The procedure of Example 3 was repeated except for using Compound-3, 7, 9, 14, 20, 26, 29, or 32 in place of Compound-1 in Example 3. In each case, good results were obtained as in Example 3; namely, precipitates were not formed in the running processing. Also, the effects of the invention were pronounced when the replenishing amount was reduced.

## EXAMPLE 5

## Preparation of Silver Halide Emulsion

To 1 liter of gelatin were added 30 g of gelatin and 6 g of potassium bromide in a container. While keeping the container at 60° C., an aqueous silver nitrate (5 g as silver nitrate) and an aqueous solution potassium bromide containing 0.15 g of potassium iodide were added to the mixture with stirring by a double jet method over a period of 1 minute. Furthermore, an aqueous silver nitrate solution (145 g as silver nitrate) and an aqueous potassium bromide solution containing 4.2 g of potassium iodide were added thereto by a double jet method. In this case, the addition flow rate of the solutions was accelerated such that the flow rate upon finishing the addition thereof was 5 times that at the beginning of the addition. Then, after removing soluble salts by a flocculation method at 35° C., the temperature was raised to 40° C., 75 g of gelatin was further added thereto, and the pH of the emulsion was adjusted to 6.7. The silver halide emulsion thus obtained contained tabular silver halide grains having a diameter of the projected area of 0.98 μm and a mean thickness of 0.138 μm, and the

content of silver iodide was 3 mol %. The silver halide emulsion was chemically sensitized using both gold sensitization and sulfur sensitization.

Preparation of Photographic Light-Sensitive Material

To prepare the surface protective layer, an aqueous gelatin solution containing gelatin, polyacrylamide having an average molecular weight of 8,000, sodium polystyrenesulfonate, polymethyl methacrylate fine particles (mean particle size 3.0  $\mu\text{m}$ ), polyethylene oxide, and a hardening agent were used.

To the foregoing silver halide emulsion were added anhydro-5,5'-dichloro-9-ethyl-3,3'-di(3-sulfopropyl)oxacarboxycyanine hydroxide sodium salt as a sensitizing dye in an amount of 500 mg/mol of Ag and potassium iodide in an amount of 200 mg/mol of Ag. Furthermore, to the emulsion were added 4-hydroxy-6-methyl-1,3,3a,7-tetraazaindene, 2,6-bis(hydroxyamino)-4-diethylamino-1,3,5-triazine, and nitron as stabilizers, trimethylolpropane as a dry antifoggant, a coating aid, and a hardening agent to provide a coating composition. The coating composition and the above-described coating composition for a surface protective layer were simultaneously coated on both surfaces of a polyethylene phthalate support to provide a photographic light-sensitive material. The coated silver amount of the photographic light-sensitive material was 2 g/m<sup>2</sup> per each surface of the support. Also, the swelling ratio according to the above-described definition was 180%.

A half of the photographic light-sensitive material was exposed to X rays with the other half of the photographic material unexposed and then processed by the developer, the fix solution and wash water shown below.

| Step        | Processing Time (sec.) | Processing Temperature (°C.) | Replenishing Amount                                                         | Tank Volume |
|-------------|------------------------|------------------------------|-----------------------------------------------------------------------------|-------------|
| Development | 13.7                   | 35                           | 20 ml (+10 ml of diluting water)                                            | 15 liters   |
| Fix         | 12.5                   | 32                           | (1) 10 ml (+30 ml of diluting water)<br>(2) 5 ml (+15 ml of diluting water) | 15 liters   |
| Wash        | 6.2                    | 20                           | 500 ml                                                                      | 10 liters   |
|             |                        |                              |                                                                             | 200 ml      |

Replenishing amount: The amount per photographic material processed (10 inches  $\times$  12 inches).

The composition of each processing solution was as

| Developer                                        | Tank Solution | Replenisher |
|--------------------------------------------------|---------------|-------------|
| Potassium Hydroxide                              | 24 g          | 60 g        |
| Sodium Sulfite                                   | 40 g          | 100 g       |
| Potassium Sulfite                                | 50 g          | 125 g       |
| Diethylenetriaminepentaacetic Acid               | 2.4 g         | 6 g         |
| Boric Acid                                       | 10 g          | 25 g        |
| Hydroquinone                                     | 35 g          | 87.5 g      |
| Diethylene Glycol                                | 11.2 g        | 28 g        |
| 4-Hydroxymethyl-4-methyl-1-phenyl-3-pyrazolidone | 2.5 g         | 6.25 g      |
| 5-Methylbenzotriazole                            | 0.06 g        | 0.15 g      |
| pH                                               | 10.05         | 11.00       |

  

| Fix Solution                                            | Tank Solution  | (1) Replenisher | (2) Replenisher |
|---------------------------------------------------------|----------------|-----------------|-----------------|
| Ammonium Thiosulfate or the compound of the Invention   | 140 g<br>1 mol | 560 g<br>4 mols | 560 g<br>4 mols |
| (Formula (I)) as shown in Table 3                       |                |                 |                 |
| Sodium Sulfite                                          | 15 g           | 60 g            | 60 g            |
| Ethylenediaminetetraacetic Acid                         | 0.025 g        | 0.1 g           | 0.1 g           |
| Disodium Salt Dihydrate                                 |                |                 |                 |
| Sodium Hydroxide                                        | 6 g<br>5.5     | 24 g<br>5.10    | 48 g<br>4.70    |
|                                                         |                |                 |                 |
| Wash Water                                              | Tank Solution  | Replenisher     |                 |
| Ethylenediaminetetraacetic Acid Disodium Salt Dihydrate | 0.5 g          | 0.5 g           |                 |

Running processing of 50 sheets (10 inches  $\times$  12 inches) of the photographic film (developing ratio for one film was 40%) per day was continued until the accumulated amount of the replenisher for the fix solution reached three times the tank volume.

When the photographic light-sensitive material was developed, the stirred liquid amount by circulation of the developer was set at 20 liters/min., and when the photographic light-sensitive material was not developed, i.e., was in a stand-by state, the stirred liquid amount was set at 6 liters/min.

After finishing running processing, the same sample as that in the running processing was processed by reducing the fixing time to 10.5 seconds or 11.5 seconds.

Also, the amount of residual silver at the unexposed portions of the processed samples was determined by a fluorescent X ray analyzer.

Also, the presence of precipitation in the fix bath was visually determined. The results obtained are shown in Table 3 below.

TABLE 3

| Fixing Agent | Replenishing Amount for Fix Bath | Residual Silver Amount ( $\mu\text{g}/\text{cm}^2$ ) |                 | Presence of Precipitation in Fix bath | Comparison |
|--------------|----------------------------------|------------------------------------------------------|-----------------|---------------------------------------|------------|
|              |                                  | Fixed 10.5 min.                                      | Fixed 11.5 min. |                                       |            |
| Ammonium     | (1)                              | 10.3                                                 | 3.2             | Δ                                     |            |
| Thiosulfate  | (2)                              | 15.5                                                 | 5.1             | X                                     |            |
| Compound-1   | (1)                              | 5.1                                                  | 0.9             | ○                                     | Invention  |
|              | (2)                              | 5.4                                                  | 1.1             | ○                                     |            |
| Compound-4   | (1)                              | 5.3                                                  | 1.0             | ○                                     | "          |
|              | (2)                              | 5.9                                                  | 1.2             | ○                                     |            |
| Compound-18  | (1)                              | 5.0                                                  | 0.8             | ○                                     | "          |
|              | (2)                              | 5.3                                                  | 0.9             | ○                                     |            |
| Compound-20  | (1)                              | 5.2                                                  | 1.0             | ○                                     | "          |
|              | (2)                              | 5.6                                                  | 1.2             | ○                                     |            |

follows.

From the results of Table 3, it can be seen that when the compound of formula (I) for use in this invention

was used, no precipitation occurred in the running processing and the liquid stability was good. Furthermore, desilvering was complete at a fixing time of 11.5 seconds, which clearly shows that the fixing ability of the compound of formula (I) of this invention is superior to that of a thiosulfate. Also the effect of this invention was particularly remarkable when the replenishing amount was reduced.

## EXAMPLE 6

The procedure of Example 5 was repeated, except that Compound-3, 5, 10, 12, 14, 19, 26 or 32 were used in place of Compound-1. In each case, good results were obtained as in Example 5; namely the fixing ability was high and precipitates were not formed in the running processing. Also, the effect of this invention was particularly remarkable when the replenishing amount was reduced.



10

Furthermore, to the emulsion were added 5-methylbenzotriazole, 4-hydroxy-1,3,3a,7-tetraazaindene, the following compounds (a) and (b), polyethylacrylate of 30% by weight to gelatin, and the following compound (c) as a gelatin hardening agent. Then, the resultant mixture was coated on a polyethylene terephthalate film of 150  $\mu\text{m}$  in thickness having a subbing layer (0.5  $\mu\text{m}$ ) composed of a vinylidene chloride copolymer at a silver coverage of 3.4  $\text{g}/\text{m}^2$ .

15



## Coating of Protective Layer

On the emulsion layer was coated a coating composition for the protective layer containing 1.5  $\text{g}/\text{m}^2$  of gelatin, polymethyl methacrylate particles (mean particle size 2.5  $\mu\text{m}$ ), and AgCl fine grains (0.08  $\mu\text{m}$ ) in an amount of 0.3  $\text{g}/\text{m}^2$  as silver using the following surface active agents.

## Surface Active Agents:



65 The sample was cut into a large area (50.8 cm  $\times$  61.0 cm). After subjecting these sheets to 50% blackening exposure with tungsten light of 3200° K., 200 sheets were processed by the following processing steps.

## EXAMPLE 7

## Preparation of Light-Sensitive Emulsion

To an aqueous gelatin solution kept at 50° C. were simultaneously added an aqueous silver nitrate solution and an aqueous solution of potassium iodide and potassium bromide in the presence of potassium iridium (III) hexachloride in an amount of  $4 \times 10^{-7}$  mol per mol of silver and ammonia, while keeping the pAg at 7.8 over a period of 60 minutes. A monodisperse emulsion was thereby obtained containing cubic silver iodobromide grains having a mean grain size of 0.28  $\mu\text{m}$  and a mean silver iodide content of 0.3 mol %. The emulsion was subjected to desalting by a flocculation method. Next, 40 g of inert gelatin per mol of silver, 5,5'-dichloro-9-ethyl-3,3'-bis(3-sulfopropyl)oxacarbocyanine as a sensitizing dye and an aqueous solution of potassium iodide of  $10^{-3}$  mol per mol of silver were added to the emulsion maintained at 50° C. The temperature was lowered after allowing the mixture to stand for 15 minutes.

## Coating of Light-Sensitive Emulsion

The emulsion was liquified and the following hydrazine derivative was added thereto at 40° C.

| Step        | Processing Step |                        |              |
|-------------|-----------------|------------------------|--------------|
|             | Processing Time | Processing Temperature | Replenisher* |
| Development | 30 sec.         | 34° C.                 | 240 ml       |
| Fix         | 30 sec.         | 34° C.                 | (1) 390 ml   |

5

Furthermore, directly before finishing the series of processing, the amount of residual silver at the unexposed portions of processed samples taken just prior to finishing the series of processing was determined by a fluorescent X-ray analyzer. The results are shown in Table 4 below.

TABLE 4

| Fixing Agent         | Replenishing Amount for Fix Bath | Residual Silver Amount ( $\mu\text{g}/\text{cm}^2$ ) | Presence of Precipitation in Fix bath |            |
|----------------------|----------------------------------|------------------------------------------------------|---------------------------------------|------------|
| Ammonium Thiosulfate | (1)                              | 0.9                                                  | Δ                                     | Comparison |
|                      | (2)                              | 3.5                                                  | x                                     |            |
| Compound-1           | (1)                              | 0.6                                                  | ○                                     | Invention  |
|                      | (2)                              | 0.9                                                  | ○                                     |            |
| Compound-4           | (1)                              | 0.6                                                  | ○                                     | "          |
|                      | (2)                              | 0.8                                                  | ○                                     |            |
| Compound-18          | (1)                              | 0.5                                                  | ○                                     | "          |
|                      | (2)                              | 0.8                                                  | ○                                     |            |
| Compound-19          | (1)                              | 0.8                                                  | ○                                     | "          |
|                      | (2)                              | 1.0                                                  | ○                                     |            |

## [Evaluation]

○: No precipitation by visual observation

Δ: Small amount of precipitation

X: Large amount of precipitation

| Wash                                                                                                              | 30 sec. | 20° C. | (2) 250 ml | 2 liters |
|-------------------------------------------------------------------------------------------------------------------|---------|--------|------------|----------|
| *The replenishing amount shown is given as the amount per square meter of the light-sensitive material processed. |         |        |            |          |

The composition of each processing solution was as follows.

| Developer                                                                   | Tank liquid = Replenisher |
|-----------------------------------------------------------------------------|---------------------------|
| Hydroquinone                                                                | 50.0 g                    |
| N-Methyl-p-aminophenol                                                      | 0.3 g                     |
| Sodium Hydroxide                                                            | 18.0 g                    |
| Boric Acid                                                                  | 20.0 g                    |
| Potassium Sulfite                                                           | 110.0 g                   |
| Ethylenediaminetetraacetic Acid                                             | 1.0 g                     |
| Disodium Salt                                                               |                           |
| Potassium Bromide                                                           | 10.0 g                    |
| 5-Methylbenzotriazole                                                       | 0.4 g                     |
| 5-Mercaptobenzimidazole-5-sulfonic Acid                                     | 0.3 g                     |
| Sodium 3-(5-Mercaptotetrazole)-benzenesulfonate                             | 0.2 g                     |
| 6-Dimethylamino-1-hexanol                                                   | 4.0 g                     |
| Sodium p-Toluenesulfonate                                                   | 15.0 g                    |
| 5-Sulfosalicylic Acid                                                       | 30.0 g                    |
| Water to make                                                               | 1 liter                   |
| pH adjusted to 11.7 with sodium hydroxide                                   |                           |
| Fix Solution                                                                | Tank liquid = Replenisher |
| Ammonium Thiosulfate or the compound of formula (I) as indicated in Table 4 | 190.0 g<br>1 mol          |
| Sodium Sulfite                                                              | 22.0 g                    |
| Ethylenediaminetetraacetic Acid                                             | 0.1 g                     |
| Disodium Salt                                                               |                           |
| Tartaric Acid                                                               | 3.0 g                     |
| Aqueous Ammonia (27 wt %)                                                   | 10.0 g                    |
| Acetic Acid (90 wt %)                                                       | 30.0 g                    |
| Aluminum Sulfate (27 wt %)                                                  | 35.0 g                    |
| Water to make                                                               | 1 liter                   |
| pH adjusted to 4.8 with sodium hydroxide                                    |                           |

After a series of continuous processing, the extent of precipitation in the fix solution was visually evaluated.

30

From the results shown in Table 4, it is clearly seen that when the compound of formula (I) of this invention is employed, the fixing ability is excellent and the fix solution has excellent liquid stability without precipitation when continuously processing a large amount of the light-sensitive material. Also, the effect of this invention was particularly remarkable when the replenishing amount was reduced.

40

The procedure of Example 7 was repeated except for using Compound-9, 13, 20 or 25 in place of Compound-1. In each case, good results were obtained as in Example 7; namely, the fixing ability was high and precipitates were not formed in the running processing. Also, the effects of the invention were pronounced when the replenishing amount was reduced.

45

By a double jet method, silver halide grains were prepared. After physical ripening and desalting treatment, the emulsion was chemically ripened to provide a silver chloroiodobromide emulsion (bromide content 30 mol %, iodide content 0.1 mol %). The mean diameter of the silver halide grains contained in the emulsion was 0.3 micron. The emulsion contained 0.6 of silver halide in 1 kg of the emulsion.

After liquifying 1 kg of the emulsion at 40° C., 70 ml of methanol solution of 0.05% by weight of the following sensitizing dye (1) was added thereto and an aqueous solution of sodium bromide was further added in a predetermined amount. Then, 25 ml of a methanol solution of 1.0% by weight of the following dye (2) was added thereto. After further adding thereto 30 ml of an aqueous solution of 1.0% by weight 1-hydroxy-3,5-dichlorotriazine sodium salt and 40 ml of an aqueous solution of sodium dodecylbenzenesulfonate, the resultant mixture was stirred.

50

55

60

65



The silver halide emulsion thus obtained was coated on a cellulose triacetate film base at a dry thickness of 5 microns followed by drying to provide a sample of the light-sensitive material.

The sample was cut into a predetermined size and subjected to a 50% blackening exposure using an actinometer having a light source of a color temperature of 2666° K. The exposed sample was subjected to running processing according to the following processing steps until the accumulated amount of the replenisher for the fix solution reached three times the tank volume thereof.

| Step        | Processing step        |                              |                          | 40 |
|-------------|------------------------|------------------------------|--------------------------|----|
|             | Processing Time (sec.) | Processing Temperature (°C.) | Replenishing Amount*     |    |
| Development | 20                     | 38                           | 320 ml                   | 18 |
| Fix         | 20                     | 38                           | (1) 320 ml<br>(2) 220 ml | 18 |
| Wash        | 20                     | 20                           | 2 liters                 | 18 |

\*Replenishing amount per square meter of the light-sensitive material processed.

The composition of each processing solution was as follows.

Developer Tank Liquid = Replenisher

-continued

|                                               |         |
|-----------------------------------------------|---------|
| Metal                                         | 0.31 g  |
| Anhydrous Sodium Sulfite                      | 39.6 g  |
| Hydroquinone                                  | 6.0 g   |
| Anhydrous Sodium Carbonate                    | 18.7 g  |
| Potassium Bromide                             | 0.86 g  |
| Citric Acid                                   | 0.68 g  |
| Potassium Metabisulfite                       | 1.5 g   |
| Water to make                                 | 1 liter |
| <u>Fix Solution Tank Liquid = Replenisher</u> |         |
| Ammonium Thiosulfate (70 wt %)                | 200 ml  |
| or the compound of formula (I)                | 1 mol   |
| as indicated in Table 5                       |         |
| Sodium Hydrogensulfite                        | 12.0 g  |
| Ethylenediaminetetraacetic                    | 0.1 g   |
| Acid Disodium Salt                            |         |
| Tartaric Acid                                 | 3.0 g   |
| Aqueous Ammonia (27 wt %)                     | 7.0 g   |
| Acetic Acid (90 wt %)                         | 20.0 g  |
| Aluminum Sulfate (27 wt %)                    | 35.0 g  |
| Water to make                                 | 1 liter |

pH of fix solution (1) was adjusted to 4.2 with sodium hydroxide and pH of fix solution (2) was adjusted to 4.0 with sodium hydroxide.

The extent of precipitation in the fix solution after running processing was completed was visually evaluated. Furthermore, the amount of residual silver at the unexposed portions of a sample taken just before the end of the running processing was determined using a fluorescent X ray analyzer. The results obtained are shown in Table 5.

TABLE 5

| Fixing Agent         | Replenishing Amount for Fix Bath | Residual Silver Amount ( $\mu\text{g}/\text{cm}^2$ ) | Presence of Precipitation in Fix bath |            |
|----------------------|----------------------------------|------------------------------------------------------|---------------------------------------|------------|
| Ammonium Thiosulfate | (1)                              | 0.8                                                  | Δ                                     | Comparison |
|                      | (2)                              | 3.1                                                  | X                                     |            |
| Compound-1           | (1)                              | 0.6                                                  | ○                                     | Invention  |
|                      | (2)                              | 0.8                                                  | ○                                     |            |
| Compound-4           | (1)                              | 0.6                                                  | ○                                     | "          |
|                      | (2)                              | 0.9                                                  | ○                                     |            |
| Compound-18          | (1)                              | 0.5                                                  | ○                                     | "          |
|                      | (2)                              | 0.7                                                  | ○                                     |            |
| Compound-26          | (1)                              | 0.6                                                  | ○                                     | "          |
|                      | (2)                              | 0.9                                                  | ○                                     |            |

[Evaluation]  
 ○: No precipitation by visual observation  
 Δ: Small amount of precipitation  
 X: Large amount of precipitation

From the results shown in Table 5, it is clearly seen that the compound of formula (I) of this invention provided a high fixing ability, and the fix solution had excellent liquid stability without precipitation when processing a large amount of the light-sensitive material. Also, the effects of the invention were pronounced when a low replenishing amount was used.

While the invention has been described in detail and with reference to specific embodiments thereof, it will be apparent to one skilled in the art that various changes and modifications can be made therein without departing from the spirit and scope thereof.

What is claimed is:

1. A process for processing an imagewise exposed silver halide photographic material comprising a support having thereon at least one light-sensitive silver halide emulsion layer, comprising the steps of developing in a developing bath and processing in a processing bath having a fixing ability containing as a fixing agent at least one compound represented by the following formula (I) in an amount of from  $2 \times 10^{-1}$  to 3 mol/l for a fixing bath and in an amount of from  $2 \times 10^{-2}$  mol/l to 10 mol/l for a bleach-fixing bath:



wherein Q represents an atomic group necessary for forming a 5- or 6-membered heterocyclic ring, which heterocyclic ring may be condensed with a carbon aromatic ring or a hetero-aromatic ring; R represents an alkyl group, an alkenyl group, an aralkyl group, an aryl group or a heterocyclic group, each group represented by R being substituted by at least one substituent selected from the group consisting of a carboxyl group or salt thereof, a sulfonic acid group or salt thereof, a phosphonic acid group or salt thereof, an amino group and an ammonium group, or R represents a single bond; n represents an integer of from 1 to 3; and M represents a cation group, wherein the processing bath having a fixing ability contains thiosulfate ion in an amount of less than 0.01 mol/l.

2. The process as in claim 1, wherein Q represents a tetrazole ring, triazole ring, imidazole ring, oxadiazole ring, triazaindene ring, tetraazaindene ring, or pentaazaindene ring; R represents an alkyl group having

from 1 to 6 carbon atoms substituted by 1 or 2 substituents selected from a carboxyl group acid or salt thereof and sulfonic acid group or salt thereof; and n represents 1 or 2.

5 3. The process as in claim 1, wherein the compound represented by formula (I) is a compound represented by formula (II):



15 wherein M and R are defined as in formula (I), T and U each represents C—R' or N; and R' represents a hydrogen atom, a halogen atom, a hydroxy group, a nitro group, an alkyl group, an alkenyl group, an aralkyl group, an aryl group, a carbonamido group, a sulfonamido group, a ureido group, a thioureido group, or R as defined in formula (I); and when R' is R as defined in formula (I), R' may be the same as or different from R of formula (II).

20 4. The process as in claim 3, wherein T and U are each N, or T and U are each C—R'; R' represents a hydrogen atom or an alkyl group having from 1 to 4 carbon atoms; and R represents an alkyl group having from 1 to 4 carbon atoms substituted by one or two substituents selected from a carboxyl group or salt thereof and a sulfonic acid group or salt thereof.

25 5. The process as in claim 1, further comprising washing in a water washing bath or stabilizing in a stabilizing bath subsequent to fixing or bleach-fixing, wherein the water washing bath or stabilizing bath contains at least one compound represented by formula (I) in a concentration of from  $10^{-3}$  to 0.5 times the concentration of the compound represented by formula (I) in the fixing bath or bleach-fixing bath.

30 6. The process as in claim 1, wherein the processing bath having a fixing ability does not contain thiosulfate ion.

35 7. The process as in claim 1, wherein the processing bath having a fixing ability does not contain a fixing agent other than the compound represented by formula (I).

\* \* \* \* \*